



US007632360B2

(12) **United States Patent**  
**Mori et al.**

(10) **Patent No.:** **US 7,632,360 B2**  
(45) **Date of Patent:** **Dec. 15, 2009**

(54) **RARE EARTH MAGNET POWDER AND METHOD OF PRODUCING THE SAME**

(75) Inventors: **Katsuhiko Mori**, Naka-gun (JP); **Ryoji Nakayama**, Naka-gun (JP); **Hideaki Ono**, Yokohama (JP); **Takae Ono**, legal representative, Yokohama (JP); **Tetsurou Tayu**, Yokosuka (JP); **Munekatsu Shimada**, Tokyo (JP); **Makoto Kano**, Yokohama (JP); **Yoshio Kawashita**, Yokosuka (JP)

(73) Assignee: **Nissan Motor Co., Ltd.**, Yokohama-shi (JP)

(\*) Notice: Subject to any disclaimer, the term of this patent is extended or adjusted under 35 U.S.C. 154(b) by 528 days.

(21) Appl. No.: **10/569,429**

(22) PCT Filed: **May 13, 2004**

(86) PCT No.: **PCT/JP2004/006784**

§ 371 (c)(1),  
(2), (4) Date: **Feb. 23, 2006**

(87) PCT Pub. No.: **WO2005/023462**

PCT Pub. Date: **Mar. 17, 2005**

(65) **Prior Publication Data**

US 2007/0079904 A1 Apr. 12, 2007

(30) **Foreign Application Priority Data**

Aug. 27, 2003 (JP) ..... 2003-209090  
Aug. 29, 2003 (JP) ..... 2003-209477

Oct. 30, 2003 (JP) ..... 2003-370054

(51) **Int. Cl.**

**H01F 1/057** (2006.01)

(52) **U.S. Cl.** ..... **148/302; 428/403; 148/101;**  
148/105; 148/122

(58) **Field of Classification Search** ..... None  
See application file for complete search history.

(56) **References Cited**

FOREIGN PATENT DOCUMENTS

|    |              |          |
|----|--------------|----------|
| EP | 0 411 571 A2 | 2/1991   |
| EP | 1 191 553 A2 | 3/2002   |
| JP | 3-129703     | 6/1991   |
| JP | 9-165601     | 6/1997   |
| JP | 2002-93610   | 3/2002   |
| JP | 2003-193208  | 7/2003   |
| JP | 2005-97711   | * 4/2005 |

\* cited by examiner

*Primary Examiner*—John P. Sheehan

(74) *Attorney, Agent, or Firm*—Kratz, Quintos & Hanson, LLP

(57) **ABSTRACT**

A rare earth magnet powder has a chemical composition which includes R: 5 to 20% (wherein, R represents one or two or more rare earth elements being inclusive of Y but exclusive of Dy and Tb), one or two of Dy and Tb: 0.01 to 10%, and B: 3 to 20%, with the balance comprising Fe and inevitable impurities; and an average particle diameter of 10 to 1,000  $\mu\text{m}$ , wherein 70% or more of the entire surface of the rare earth magnet powder is covered with a layer being rich in the content of one or two of Dy and Tb and having a thickness of 0.05 to 50  $\mu\text{m}$ .

**7 Claims, 5 Drawing Sheets**



FIG. 1



FIG. 2



FIG. 3



FIG. 4



FIG. 5



FIG. 6



FIG. 7



## 1

RARE EARTH MAGNET POWDER AND  
METHOD OF PRODUCING THE SAME

## TECHNICAL FIELD

The present invention relates to a rare earth magnet powder which is excellent in magnetic anisotropy and thermal stability and method of producing the same.

## BACKGROUND ART

A known method of producing a rare earth magnet powder which is excellent in magnetic anisotropy includes mixing a rare earth magnet alloy raw material hydride powder having a chemical composition which includes, in atom % (hereinafter % represents atom %), one, or two or more rare earth element including Y: 10 to 20%, Co: 0 to 50%, B: 3 to 20%, and M: 0 to 5% (wherein M represents one, or two or more from among Ga, Zr, Nb, Mo, Hf, Ta, W, Ni, Al, Ti, V, Cu, Cr, Ge, C, and Si), with the balance including Fe and inevitable impurities, and a powder including Dy and Tb in an elemental, alloy, or compound form, or in hydrides thereof (an elemental, alloy, or compound form) so as to produce a mixed powder; diffusion heat-treating the mixed powder; and then carrying out hydrogen absorption of the diffusion heat-treated mixed powder.

The aforementioned rare earth magnet alloy raw material hydride powder is produced by the following known method: carrying out hydrogen absorption by heating, or heating and holding a rare earth magnet alloy raw material from room temperature to a temperature below 500° C. in a hydrogen atmosphere; carrying out hydrogen absorption-decomposition by heating and holding the rare earth magnet alloy raw material at a predetermined temperature in a range of 500 to 1,000° C. in a hydrogen atmosphere with a pressure of 10 to 1,000 kPa so as to induce the rare earth magnet alloy raw material to absorb hydrogen and to be decomposed due to a phase transformation; carrying out heat treatment in depressurized hydrogen with some hydrogen remaining in the rare earth magnet alloy raw material by holding the rare earth magnet alloy raw material subjected to the hydrogen absorption-decomposition at a predetermined temperature in a range of 500 to 1,000° C. in a hydrogen atmosphere with an absolute pressure of at least 0.65 but less than 10 kPa or in a mixed hydrogen/inert gas atmosphere with a hydrogen partial pressure of at least 0.65 but less than 10 kPa; and then cooling the rare earth magnet alloy raw material to room temperature by introducing Ar gas (see Patent document 1: Japanese Patent Application, First Publication No. 2002-93610).

Also, in the case of producing a magnetically anisotropic HDDR magnet powder that is the aforementioned rare earth magnet powder, the following method is used: carrying out hydrogen absorption for a rare earth magnet alloy raw material; carrying out hydrogen absorption-decomposition by heating and holding the rare earth magnet alloy raw material at a predetermined temperature in a range of 500 to 1,000° C. in a hydrogen atmosphere with a pressure of 10 to 1,000 kPa so as to induce the rare earth magnet alloy raw material to absorb hydrogen and to be decomposed due to a phase transformation; and then carrying out hydrogen desorption by holding the rare earth magnet alloy raw material subjected to the hydrogen absorption at a predetermined temperature in a range of 500 to 1,000° C. in vacuum. Accordingly, the magnet obtained by the aforementioned method is known to have a recrystallization texture in which recrystallized grains, whose main phase is a  $R_2Fe_{14}B$  intermetallic compound phase that is substantially a tetragonal structure, are adjacent to each other, and the recrystallization texture includes a basic texture of a

## 2

magnetically anisotropic HDDR magnet powder in which the recrystallized grains, whose ratio (b/a) of a longest particle diameter (b) to a shortest particle diameter (a) is less than 2, exists at 50 vol % or more of all the recrystallized grains and an average recrystallized grain diameter of the recrystallized grains is 0.05 to 5  $\mu m$  (see Patent document 2: Japanese Patent No. 2576672).

Recently, in the electrical and electronics industries, a need has arisen for a rare earth magnet powder which is further excellent in magnetic anisotropy. In the automotive industry in particular, active development work is being carried out on electric vehicles, including the motors to be mounted in such vehicles. The motors that are mounted in such electric vehicles are sometimes installed close to a small gasoline engine or left out under the scorching sun, so it is not unusual for them to be placed in an environment where they are particularly subjected to heating. Accordingly, there exists a need for a rare earth magnet powder which is so excellent in thermal stability and magnetic anisotropy including both coercivity and remanence that it can be used to produce motor components which is further excellent in heat resistance and magnetic properties.

## DISCLOSURE OF INVENTION

The present inventors have conducted research with the aim of obtaining a rare earth magnet powder which is further excellent in magnetic anisotropy and thermal stability. In consequence, the research results described in (i) to (iii) below were obtained.

(i) (a) A rare earth magnet powder having a chemical composition which includes, in atom % (hereinafter % represents atom %), R: 5 to 20% (wherein R represents one, or two or more rare earth elements being inclusive of Y but exclusive of Dy and Tb; the same applies below), one or both of Dy and Tb: 0.01 to 10%, and B: 3 to 20%, with the balance including Fe and inevitable impurities, an average particle diameter being 10 to 1,000  $\mu m$ , wherein 70% or more of the entire surface of the rare earth magnet powder is covered with a layer being rich in content of the one or both of Dy and Tb and having a thickness of 0.05 to 50  $\mu m$  (hereinafter referred to as a "Dy—Tb rich layer"), and a concentration of the one or both of Dy and Tb in the Dy—Tb rich layer is such that the maximum detected intensity of the one or both of Dy and Tb, as measured by wavelength dispersive X-ray spectroscopy, is 1.2 to 5 times the average detected intensity in the central portion being present in the range of  $1/3$  of the particle diameter of a particle of the rare earth magnet powder.

(b) A rare earth magnet powder having a chemical composition which includes R: 5 to 20%, one or both of Dy and Tb: 0.01 to 10%, B: 3 to 20%, and M: 0.001 to 5% (wherein M represents one, or two or more from among Ga, Zr, Nb, Mo, Hf, Ta, W, Ni, Al, Ti, V, Cu, Cr, Ge, C, and Si), with the balance including Fe and inevitable impurities, an average particle diameter being 10 to 1,000  $\mu m$ , wherein 70% or more of the entire surface of the rare earth magnet powder is covered with a Dy—Tb rich layer being rich in content of the one or both of Dy and Tb and having a thickness of 0.05 to 50  $\mu m$ , and a concentration of the one or both of Dy and Tb in the Dy—Tb rich layer is such that the maximum detected intensity of the one or both of Dy and Tb, as measured by wavelength dispersive X-ray spectroscopy, is 1.2 to 5 times the average detected intensity in the central portion being present in the range of  $1/3$  of the particle diameter of a particle of the rare earth magnet powder.

(c) A rare earth magnet powder having a chemical composition which includes R: 5 to 20%, Co: 0.1 to 50%, one or both

of Dy and Tb: 0.01 to 10%, and B: 3 to 20%, with the balance including Fe and inevitable impurities, an average particle diameter being 10 to 1,000  $\mu\text{m}$ , wherein 70% or more of the entire surface of the rare earth magnet powder is covered with a Dy—Tb rich layer being rich in content of the one or both of Dy and Tb and having a thickness of 0.05 to 50  $\mu\text{m}$ , and a concentration of the one or both of Dy and Tb in the Dy—Tb rich layer is such that the maximum detected intensity of the one or both of Dy and Tb, as measured by wavelength dispersive X-ray spectroscopy, is 1.2 to 5 times the average detected intensity in the central portion being present in the range of  $\frac{1}{3}$  of the particle diameter of a particle of the rare earth magnet powder.

(d) A rare earth magnet powder having a chemical composition which includes R: 5 to 20%, Co: 0.1 to 50%, one or both of Dy and Tb: 0.01 to 10%, and B: 3 to 20%, with the balance including Fe and inevitable impurities, an average particle diameter being 10 to 1,000  $\mu\text{m}$ , wherein 70% or more of the entire surface of the rare earth magnet powder is covered with a Dy—Tb rich layer being rich in content of the one or both of Dy and Tb and having a thickness of 0.05 to 50  $\mu\text{m}$ , and a concentration of the one or both of Dy and Tb in the Dy—Tb rich layer is such that the maximum detected intensity of the one or both of Dy and Tb, as measured by wavelength dispersive X-ray spectroscopy, is 1.2 to 5 times the average detected intensity in the central portion being present in the range of  $\frac{1}{3}$  of the particle diameter of a particle of the rare earth magnet powder.

Each of the rare earth magnet powders described in (a) to (d) above is further excellent in magnetic anisotropy and thermal stability than the conventional rare earth magnet powder described in Patent document 1.

(ii) Each of the rare earth magnet powders has a recrystallization texture in which recrystallized grains, whose main phase is a  $\text{R}_2\text{Fe}_{14}\text{B}$  intermetallic compound phase that is substantially a tetragonal structure, are adjacent to each other, and the recrystallization texture includes a basic texture of a magnetically anisotropic HDDR magnet powder in which the recrystallized grains, whose ratio (b/a) of a longest particle diameter (b) to a shortest particle diameter (a) is less than 2, exists at 50 vol % or more of all the recrystallized grains and an average recrystallized grain diameter of the recrystallized grains is 0.05 to 5  $\mu\text{m}$ .

(iii) These rare earth magnet powders having magnetic anisotropy and thermal stability can be used to produce rare earth magnets by conventional methods.

For the purpose of producing the aforementioned rare earth magnet powders which are further excellent magnetic anisotropy and thermal stability, (A) the following steps are used in the aforementioned conventional method of producing a rare earth magnet powder which is excellent in magnetic anisotropy: milling a rare earth magnet alloy raw material in a conventional inert gas atmosphere to an average powder particle diameter of 10 to 1,000  $\mu\text{m}$  so as to produce a rare earth magnet alloy raw material powder; adding to the rare earth magnet alloy raw material powder a Dy hydride powder, a Tb hydride powder, or a Dy—Tb binary alloy hydride powder, each of which has an average powder particle diameter of 0.1 to 50  $\mu\text{m}$ , at 0.01 to 5 mol %, followed by mixing so as to produce a mixed powder; carrying out hydrogen absorption by heating, or heating and holding the mixed powder from room temperature to a temperature below 500° C. in a hydrogen gas atmosphere with a pressure of 10 to 1,000 kPa so as to induce the mixed powder to absorb hydrogen; and then carrying out hydrogen absorption-decomposition by heating and holding the mixed powder at a temperature in a range of 500 to 1,000° C. in a hydrogen gas atmosphere with a pressure of

10 to 1,000 kPa so as to induce the mixed powder to absorb hydrogen and to be decomposed. Subsequently, as in the case of the conventional method, the following steps are used if necessary: carrying out intermediate heat treatment by holding the mixed powder subjected to the hydrogen absorption-decomposition at a predetermined temperature in a range of 500 to 1,000° C. in an inert gas atmosphere with an inert gas pressure of 10 to 1,000 kPa; and/or carrying out heat treatment in depressurized hydrogen with some hydrogen remaining in the mixed powder by holding the mixed powder subjected to the intermediate heat treatment at a predetermined temperature in a range of 500 to 1,000° C. in a hydrogen atmosphere with an absolute pressure of at least 0.65 but less than 10 kPa or in a mixed hydrogen/inert gas atmosphere with a hydrogen partial pressure of at least 0.65 but less than 10 kPa. Finally, the following step is used: carrying out hydrogen desorption by holding the mixed powder at a temperature in a range of 500 to 1,000° C. in a vacuum atmosphere with an ultimate pressure of 0.13 kPa or below so as to forcibly release hydrogen and promote a phase transformation, followed by cooling and pulverizing, thereby producing the aforementioned rare earth magnet powders which are further excellent magnetic anisotropy and thermal stability.

(B) Alternatively, the following steps are used: if necessary, subjecting a rare earth magnet alloy raw material to hydrogen absorption by heating, or heating and holding the rare earth magnet alloy raw material from room temperature to a temperature below 500° C. in a hydrogen gas atmosphere with a pressure of 10 to 1,000 kPa so as to induce the rare earth magnet alloy raw material to absorb hydrogen; milling the hydrogen-absorbing rare earth magnet alloy raw material to an average powder particle diameter of 10 to 1,000  $\mu\text{m}$  so as to produce a rare earth magnet alloy raw material powder subjected to the hydrogen absorption (hereinafter referred to as a “hydrogen-absorbing rare earth magnet alloy raw material powder”); adding to a hydrogen-absorbing rare earth magnet alloy raw material powder a Dy hydride powder, a Tb hydride powder, or a Dy—Tb binary alloy hydride powder, each of which has an average powder particle diameter of 0.1 to 50  $\mu\text{m}$ , at 0.01 to 5 mol %, followed by mixing so as to produce a hydrogen-containing raw material mixed powder; and then carrying out hydrogen absorption-decomposition by heating and holding the hydrogen-containing raw material mixed powder at a temperature in a range of 500 to 1,000° C. in a hydrogen gas atmosphere with a pressure of 10 to 1,000 kPa so as to induce the hydrogen-containing raw material mixed powder to absorb further hydrogen and to be decomposed. Subsequently, the following steps are used if necessary: carrying out intermediate heat treatment by holding the hydrogen-containing raw material mixed powder subjected to the hydrogen absorption-decomposition at a temperature in a range of 500 to 1,000° C. in an inert gas atmosphere with a pressure of 10 to 1,000 kPa; and/or carrying out heat treatment in depressurized hydrogen with some hydrogen remaining in the hydrogen-containing raw material mixed powder by holding the hydrogen-containing raw material mixed powder subjected to the intermediate heat treatment at a temperature in a range of 500 to 1,000° C. in a hydrogen atmosphere with an absolute pressure of at least 0.65 but less than 10 kPa or in a mixed hydrogen/inert gas atmosphere with a hydrogen partial pressure of at least 0.65 but less than 10 kPa. Finally, the following step is used: carrying out hydrogen desorption by holding the hydrogen-containing raw material mixed powder at a temperature in a range of 500 to 1,000° C. in a vacuum atmosphere with an ultimate pressure of 0.13 kPa or below so as to forcibly release hydrogen and promote a phase transformation, followed by cooling and pulverizing, so as to be able

to produce the rare earth magnet powders which are further excellent magnetic anisotropy and thermal stability.

It is preferable that the aforementioned rare earth magnet alloy raw material has a chemical composition, in atom % (hereinafter % represents atom %), including R': 10 to 20% (wherein R' represents one, or two or more rare earth elements being inclusive of Y but exclusive of Dy and Tb; the same applies below) and B: 3 to 20%, with the balance including Fe and inevitable impurities; a chemical composition including R': 10 to 20%, B: 3 to 20%, and M: 0.001 to 5% (wherein M represents one, or two or more from among Ga, Zr, Nb, Mo, Hf, Ta, W, Ni, Al, Ti, V, Cu, Cr, Ge, C, and Si), with the balance including Fe and inevitable impurities; a chemical composition including R': 10 to 20%, Co: 0.1 to 50%, and B: 3 to 20%, with the balance including Fe and inevitable impurities; or a chemical composition including R': 10 to 20%, Co: 0.1 to 50%, B: 3 to 20%, and M: 0.001 to 5%, with the balance including Fe and inevitable impurities.

The present invention was achieved on the basis on these research results, and is characterized in the following.

(1) A rare earth magnet powder having a chemical composition which includes, in atom % (hereinafter % represents atom %), R: 5 to 20% (wherein R represents one, or two or more rare earth elements being inclusive of Y but exclusive of Dy and Tb; the same applies below), one or both of Dy and Tb: 0.01 to 10%, and B: 3 to 20%, with the balance including Fe and inevitable impurities, an average particle diameter being 10 to 1,000  $\mu\text{m}$ , wherein 70% or more of the entire surface of the rare earth magnet powder is covered with a layer being rich in content of the one or both of Dy and Tb and having a thickness of 0.05 to 50  $\mu\text{m}$  (hereinafter referred to as a "Dy—Tb rich layer"), and a concentration of the one or both of Dy and Tb in the Dy—Tb rich layer is such that the maximum detected intensity of the one or both of Dy and Tb, as measured by wavelength dispersive X-ray spectroscopy, is 1.2 to 5 times the average detected intensity in the central portion being present in the range of  $\frac{1}{3}$  of the particle diameter of a particle of the rare earth magnet powder.

(2) A rare earth magnet powder having a chemical composition which includes R: 5 to 20%, one or both of Dy and Tb: 0.01 to 10%, B: 3 to 20%, and M: 0.001 to 5% (wherein M represents one, or two or more from among Ga, Zr, Nb, Mo, Hf, Ta, W, Ni, Al, Ti, V, Cu, Cr, Ge, C, and Si), with the balance including Fe and inevitable impurities, an average particle diameter being 10 to 1,000  $\mu\text{m}$ , wherein 70% or more of the entire surface of the rare earth magnet powder is covered with a Dy—Tb rich layer being rich in content of the one or both of Dy and Tb and having a thickness of 0.05 to 50  $\mu\text{m}$ , and a concentration of the one or both of Dy and Tb in the Dy—Tb rich layer is such that the maximum detected intensity of the one or both of Dy and Tb, as measured by wavelength dispersive X-ray spectroscopy, is 1.2 to 5 times the average detected intensity in the central portion being present in the range of  $\frac{1}{3}$  of the particle diameter of a particle of the rare earth magnet powder.

(3) A rare earth magnet powder having a chemical composition which includes R: 5 to 20%, Co: 0.1 to 50%, one or both of Dy and Tb: 0.01 to 10%, and B: 3 to 20%, with the balance including Fe and inevitable impurities, an average particle diameter being 10 to 1,000  $\mu\text{m}$ , wherein 70% or more of the entire surface of the rare earth magnet powder is covered with a Dy—Tb rich layer being rich in content of the one or both of Dy and Tb and having a thickness of 0.05 to 50  $\mu\text{m}$ , and a concentration of the one or both of Dy and Tb in the Dy—Tb rich layer is such that the maximum detected intensity of the one or both of Dy and Tb, as

measured by wavelength dispersive X-ray spectroscopy, is 1.2 to 5 times the average detected intensity in the central portion being present in the range of  $\frac{1}{3}$  of the particle diameter of a particle of the rare earth magnet powder.

- 5 (4) A rare earth magnet powder having a chemical composition which includes R: 5 to 20%, one or both of Dy and Tb: 0.01 to 10%, Co: 0.1 to 50%, B: 3 to 20%, and M: 0.001 to 5%, with the balance including Fe and inevitable impurities, an average particle diameter being 10 to 1,000  $\mu\text{m}$ , wherein 70% or more of the entire surface of the rare earth magnet powder is covered with a Dy—Tb rich layer being rich in content of the one or both of Dy and Tb and having a thickness of 0.05 to 50  $\mu\text{m}$ , and a concentration of the one or both of Dy and Tb in the Dy—Tb rich layer is such that the maximum detected intensity of the one or both of Dy and Tb, as measured by wavelength dispersive X-ray spectroscopy, is 1.2 to 5 times the average detected intensity in the central portion being present in the range of  $\frac{1}{3}$  of the particle diameter of a particle of the rare earth magnet powder.
- 10 (5) A rare earth magnet produced by binding a rare earth magnet powder which is excellent in magnetic anisotropy and thermal stability according to any one of claims (1) to (4) with an organic binder or a metal binder.
- 15 (6) A rare earth magnet produced by processing a rare earth magnet powder which is excellent in magnetic anisotropy and thermal stability according to any one of claims (1) to (4) with hot pressing or hot isostatic pressing.
- 20 (7) A method of producing a rare earth magnet powder, including: milling a rare earth magnet alloy raw material in an inert gas atmosphere to an average powder particle diameter of 10 to 1,000  $\mu\text{m}$  so as to produce a rare earth magnet alloy raw material powder; adding to the rare earth magnet alloy raw material powder a Dy hydride powder, a Tb hydride powder, or a Dy—Tb binary alloy hydride powder, each of which has an average powder particle diameter of 0.1 to 50  $\mu\text{m}$ , at 0.01 to 5 mol %, followed by mixing so as to produce a mixed powder; carrying out hydrogen absorption by heating, or heating and holding the mixed powder from room temperature to a temperature below 500° C. in a hydrogen gas atmosphere with a pressure of 10 to 1,000 kPa so as to induce the mixed powder to absorb hydrogen; carrying out hydrogen absorption-decomposition by heating and holding the mixed powder at a temperature in a range of 500 to 1,000° C. in a hydrogen gas atmosphere with a pressure of 10 to 1,000 kPa so as to induce the mixed powder to absorb hydrogen and to be decomposed; and then carrying out hydrogen desorption by holding the mixed powder at a temperature in a range of 500 to 1,000° C. in a vacuum atmosphere with an ultimate pressure of 0.13 kPa or below so as to forcibly release hydrogen and promote a phase transformation, followed by cooling and pulverizing.
- 25 (8) A method of producing a rare earth magnet powder, including: milling a rare earth magnet alloy raw material in an inert gas atmosphere to an average powder particle diameter of 10 to 1,000  $\mu\text{m}$  so as to produce a rare earth magnet alloy raw material powder; adding to the rare earth magnet alloy raw material powder a Dy hydride powder, a Tb hydride powder, or a Dy—Tb binary alloy hydride powder, each of which has an average powder particle diameter of 0.1 to 50  $\mu\text{m}$ , at 0.01 to 5 mol %, followed by mixing so as to produce a mixed powder; carrying out hydrogen absorption by heating, or heating and holding the mixed powder from room temperature to a temperature below 500° C. in a hydrogen gas atmosphere with a pressure of 10 to 1,000 kPa so as to induce the mixed powder to

absorb hydrogen; carrying out hydrogen absorption-decomposition by heating and holding the mixed powder at a temperature in a range of 500 to 1,000° C. in a hydrogen gas atmosphere with a pressure of 10 to 1,000 kPa so as to induce the mixed powder to absorb hydrogen and to be decomposed; carrying out intermediate heat treatment by holding the mixed powder subjected to the hydrogen absorption-decomposition at a temperature in a range of 500 to 1,000° C. in an inert gas atmosphere with a pressure of 10 to 1,000 kPa; and then carrying out hydrogen desorption by holding the powder at a temperature in a range of 500 to 1,000° C. in a vacuum atmosphere with an ultimate pressure of 0.13 kPa or below so as to forcibly release hydrogen and promote a phase transformation, followed by cooling and pulverizing.

(9) A method of producing a rare earth magnet powder, including: milling a rare earth magnet alloy raw material in an inert gas atmosphere to an average powder particle diameter of 10 to 1,000  $\mu\text{m}$  so as to produce a rare earth magnet alloy raw material powder; adding to the rare earth magnet alloy raw material powder a Dy hydride powder, a Tb hydride powder, or a Dy—Tb binary alloy hydride powder, each of which has an average powder particle diameter of 0.1 to 50  $\mu\text{m}$ , at 0.01 to 5 mol %, followed by mixing so as to produce a mixed powder; carrying out hydrogen absorption by heating, or heating and holding the mixed powder from room temperature to a temperature below 500° C. in a hydrogen gas atmosphere with a pressure of 10 to 1,000 kPa so as to induce the mixed powder to absorb hydrogen; carrying out hydrogen absorption-decomposition by heating and holding the mixed powder at a temperature in a range of 500 to 1,000° C. in a hydrogen gas atmosphere with a pressure of 10 to 1,000 kPa so as to induce the mixed powder to absorb hydrogen and to be decomposed; carrying out heat treatment in depressurized hydrogen with some hydrogen remaining in the mixed powder by holding the mixed powder subjected to the hydrogen absorption-decomposition at a temperature in a range of 500 to 1,000° C. in a hydrogen atmosphere with an absolute pressure of at least 0.65 but less than 10 kPa or in a mixed hydrogen/inert gas atmosphere with a hydrogen partial pressure of at least 0.65 but less than 10 kPa; and then carrying out hydrogen desorption by holding the powder at a temperature in a range of 500 to 1,000° C. in a vacuum atmosphere with an ultimate pressure of 0.13 kPa or below so as to forcibly release hydrogen and promote a phase transformation, followed by cooling and pulverizing.

(10) A method of producing a rare earth magnet powder, including: milling a rare earth magnet alloy raw material in an inert gas atmosphere to an average powder particle diameter of 10 to 1,000  $\mu\text{m}$  so as to produce a rare earth magnet alloy raw material powder; adding to the rare earth magnet alloy raw material powder a Dy hydride powder, a Tb hydride powder, or a Dy—Tb binary alloy hydride powder, each of which has an average powder particle diameter of 0.1 to 50  $\mu\text{m}$ , at 0.01 to 5 mol %, followed by mixing so as to produce a mixed powder; carrying out hydrogen absorption by heating, or heating and holding the mixed powder from room temperature to a temperature below 500° C. in a hydrogen gas atmosphere with a pressure of 10 to 1,000 kPa so as to induce the mixed powder to absorb hydrogen; carrying out hydrogen absorption-decomposition by heating and holding the mixed powder at a temperature in a range of 500 to 1,000° C. in a hydrogen gas atmosphere with a pressure of 10 to 1,000 kPa so as to induce the mixed powder to absorb hydrogen and to be

decomposed; carrying out intermediate heat treatment by holding the mixed powder subjected to the hydrogen absorption-decomposition at a temperature in a range of 500 to 1,000° C. in an inert gas atmosphere with a pressure of 10 to 1,000 kPa; carrying out heat treatment in depressurized hydrogen with some hydrogen remaining in the mixed powder by holding the mixed powder subjected to the intermediate heat treatment at a temperature in a range of 500 to 1,000° C. in a hydrogen atmosphere with an absolute pressure of at least 0.65 but less than 10 kPa or in a mixed hydrogen/inert gas atmosphere with a hydrogen partial pressure of at least 0.65 but less than 10 kPa; and then carrying out hydrogen desorption by holding the powder at a temperature in a range of 500 to 1,000° C. in a vacuum atmosphere with an ultimate pressure of 0.13 kPa or below so as to forcibly release hydrogen and promote a phase transformation, followed by cooling and pulverizing.

(11) A method of producing a rare earth magnet powder according to any one of (7) to (10), wherein the rare earth magnet alloy raw material has been homogenized by holding in a vacuum or Ar gas atmosphere at a temperature of 600 to 1,200° C.

(12) A method of producing a rare earth magnet powder, including: subjecting a rare earth magnet alloy raw material to hydrogen absorption by heating, or heating and holding the rare earth magnet alloy raw material from room temperature to a temperature below 500° C. in a hydrogen gas atmosphere with a pressure of 10 to 1,000 kPa so as to induce the rare earth magnet alloy raw material to absorb hydrogen; milling the hydrogen-absorbing rare earth magnet alloy raw material to an average powder particle diameter of 10 to 1,000  $\mu\text{m}$  so as to produce a rare earth magnet alloy raw material powder subjected to the hydrogen absorption (hereinafter referred to as a “hydrogen-absorbing rare earth magnet alloy raw material powder”); adding to the hydrogen-absorbing rare earth magnet alloy raw material powder a Dy hydride powder, a Tb hydride powder, or a Dy—Tb binary alloy hydride powder, each of which has an average powder particle diameter of 0.1 to 50  $\mu\text{m}$ , at 0.01 to 5 mol %, followed by mixing so as to produce a hydrogen-containing raw material mixed powder; carrying out hydrogen absorption-decomposition by heating and holding the hydrogen-containing raw material mixed powder at a temperature in a range of 500 to 1,000° C. in a hydrogen gas atmosphere with a pressure of 10 to 1,000 kPa so as to induce the hydrogen-containing raw material mixed powder to absorb further hydrogen and to be decomposed; and then carrying out hydrogen desorption by holding the hydrogen-containing raw material mixed powder at a temperature in a range of 500 to 1,000° C. in a vacuum atmosphere with an ultimate pressure of 0.13 kPa or below so as to forcibly release hydrogen and promote a phase transformation, followed by cooling and pulverizing.

(13) A method of producing a rare earth magnet powder, including: adding to a hydrogen-absorbing rare earth magnet alloy raw material powder a Dy hydride powder, a Tb hydride powder, or a Dy—Tb binary alloy hydride powder, each of which has an average powder particle diameter of 0.1 to 50  $\mu\text{m}$ , at 0.01 to 5 mol %, followed by mixing so as to produce a hydrogen-containing raw material mixed powder; carrying out hydrogen absorption-decomposition by heating and holding the hydrogen-containing raw material mixed powder at a temperature in a range of 500 to 1,000° C. in a hydrogen gas atmosphere with a pressure of 10 to 1,000 kPa so as to induce the hydrogen-containing raw material mixed powder to absorb further hydrogen and

to be decomposed; carrying out intermediate heat treatment by holding the hydrogen-containing raw material mixed powder subjected to the hydrogen absorption-decomposition at a temperature in a range of 500 to 1,000° C. in an inert gas atmosphere with a pressure of 10 to 1,000 kPa; and then carrying out hydrogen desorption by holding the hydrogen-containing raw material mixed powder at a temperature in a range of 500 to 1,000° C. in a vacuum atmosphere with an ultimate pressure of 0.13 kPa or below so as to forcibly release hydrogen and promote a phase transformation, followed by cooling and pulverizing.

(14) A method of producing a rare earth magnet powder, including: adding to a hydrogen-absorbing rare earth magnet alloy raw material powder a Dy hydride powder, a Tb hydride powder, or a Dy—Tb binary alloy hydride powder, each of which has an average powder particle diameter of 0.1 to 50  $\mu\text{m}$ , at 0.01 to 5 mol %, followed by mixing so as to produce a hydrogen-containing raw material mixed powder; carrying out hydrogen absorption-decomposition by heating and holding the hydrogen-containing raw material mixed powder at a temperature in a range of 500 to 1,000° C. in a hydrogen gas atmosphere with a pressure of 10 to 1,000 kPa so as to induce the hydrogen-containing raw material mixed powder to absorb further hydrogen and to be decomposed; carrying out heat treatment in depressurized hydrogen with some hydrogen remaining in the hydrogen-containing raw material mixed powder by holding the hydrogen-containing raw material mixed powder subjected to the hydrogen absorption-decomposition at a temperature in a range of 500 to 1,000° C. in a hydrogen atmosphere with an absolute pressure of at least 0.65 but less than 10 kPa or in a mixed hydrogen/inert gas atmosphere with a hydrogen partial pressure of at least 0.65 but less than 10 kPa; and then carrying out hydrogen desorption by holding the hydrogen-containing raw material mixed powder at a temperature in a range of 500 to 1,000° C. in a vacuum atmosphere with an ultimate pressure of 0.13 kPa or below so as to forcibly release hydrogen and promote a phase transformation, followed by cooling and pulverizing.

(15) A method of producing a rare earth magnet powder, including: adding to a hydrogen-absorbing rare earth magnet alloy raw material powder a Dy hydride powder, a Tb hydride powder, or a Dy—Tb binary alloy hydride powder, each of which has an average powder particle diameter of 0.1 to 50  $\mu\text{m}$ , at 0.01 to 5 mol %, followed by mixing so as to produce a hydrogen-containing raw material mixed powder; carrying out hydrogen absorption-decomposition by heating and holding the hydrogen-containing raw material mixed powder at a temperature in a range of 500 to 1,000° C. in a hydrogen gas atmosphere with a pressure of 10 to 1,000 kPa so as to induce the hydrogen-containing raw material mixed powder to absorb further hydrogen and to be decomposed; carrying out intermediate heat treatment by holding the hydrogen-containing raw material mixed powder subjected to the hydrogen absorption-decomposition at a temperature in a range of 500 to 1,000° C. in an inert gas atmosphere with a pressure of 10 to 1,000 kPa; and then carrying out heat treatment in depressurized hydrogen with some hydrogen remaining in the hydrogen-containing raw material mixed powder by holding the hydrogen-containing raw material mixed powder subjected to the intermediate heat treatment at a temperature in a range of 500 to 1,000° C. in a hydrogen atmosphere with an absolute pressure of at least 0.65 but less than 10 kPa or in a mixed hydrogen/inert gas atmosphere with a hydrogen partial pressure of at least 0.65 but less than 10 kPa; and

then carrying out hydrogen desorption by holding the hydrogen-containing raw material mixed powder at a temperature in a range of 500 to 1,000° C. in a vacuum atmosphere with an ultimate pressure of 0.13 kPa or below so as to forcibly release hydrogen and promote a phase transformation, followed by cooling and pulverizing.

(16) A method of producing a rare earth magnet powder according to any one of (12) to (15), wherein a rare earth magnet alloy raw material for producing the hydrogen-absorbing rare earth magnet alloy raw material powder has been homogenized by holding in a vacuum or Ar gas atmosphere at a temperature of 600 to 1,200° C.

(17) A method of producing a rare earth magnet, including binding a rare earth magnet powder which is excellent in magnetic anisotropy and thermal stability produced by the method according to any one of (7) to (16) with an organic binder or a metal binder.

(18) A method of producing a rare earth magnet, including: molding a rare earth magnet powder which is excellent in magnetic anisotropy and thermal stability produced by the method according to any one of (7) to (16) so as to produce a green compact; and processing the green compact with hot pressing or hot isostatic pressing at a temperature of 600 to 900° C.

(19) A method of producing a rare earth magnet powder according to any one of (7) to (16), wherein the rare earth magnet alloy raw material has: a chemical composition, in atom % (hereinafter % represents atom %), including R': 10 to 20% (wherein R' represents one, or two or more rare earth elements being inclusive of Y but exclusive of Dy and Tb; the same applies below) and B: 3 to 20%, with the balance including Fe and inevitable impurities; a chemical composition including R': 10 to 20%, B: 3 to 20%, and M: 0.001 to 5% (wherein M represents one, or two or more from among Ga, Zr, Nb, Mo, Hf, Ta, W, Ni, Al, Ti, V, Cu, Cr, Ge, C, and Si), with the balance including Fe and inevitable impurities; a chemical composition including R': 10 to 20%, Co: 0.1 to 50%, and B: 3 to 20%, with the balance including Fe and inevitable impurities; or a chemical composition including R': 10 to 20%, Co: 0.1 to 50%, B: 3 to 20%, and M: 0.001 to 5%, with the balance including Fe and inevitable impurities.

Rare earth magnet powders obtained by the methods of producing a rare earth magnet powder of the present invention, which includes, in order, producing a rare earth magnet alloy raw material powder or a hydrogen-absorbing rare earth magnet alloy raw material powder; adding to the rare earth magnet alloy raw material powder a Dy hydride powder, a Tb hydride powder, or a Dy—Tb binary alloy hydride powder at 0.01 to 5 mol %, followed by mixing so as to produce a mixed powder; hydrogen absorption; hydrogen absorption-decomposition; optional intermediate heat treatment; optional heat treatment in depressurized hydrogen; and then hydrogen desorption, are excellent in magnetic anisotropy and thermal stability, and thus exhibits industrially advantageous effects.

#### BRIEF DESCRIPTION OF THE DRAWINGS

FIG. 1 is an elemental distribution image obtained by using an electron probe microanalyzer (EPMA), which shows the elemental distribution of Dy contained in the anisotropic magnet powder produced by the present invention's method 1.

FIG. 2 is a line analysis graph obtained by using an electron probe microanalyzer (EPMA), which shows the distribution

## 11

of Dy on line A-B in FIG. 1 of Dy contained in the anisotropic magnet powder produced by the present invention's method 1.

FIG. 3 is a line analysis graph obtained by scanning at fine intervals near peak A in FIG. 2, which shows the elemental distribution on the line of Dy contained in the anisotropic magnet powder produced by the present invention's method 1.

FIG. 4 is a line analysis graph obtained by using an electron probe microanalyzer (EPMA), which shows the elemental distribution of Dy contained in the anisotropic magnet powder produced by the conventional method 1.

FIG. 5 is a line analysis graph obtained by scanning at fine intervals near peak C in FIG. 4, which shows the elemental distribution of Dy contained in the anisotropic magnet powder produced by the conventional method 1.

FIG. 6 is an elemental distribution image obtained by using an electron probe microanalyzer (EPMA), which shows the elemental distribution of Dy contained in the anisotropic magnet powder produced by the present invention's method 16.

FIG. 7 is a line analysis graph obtained by using an electron probe microanalyzer (EPMA), which shows the distribution of Dy on line E-F in FIG. 6 of Dy contained in the anisotropic magnet powder produced by the present invention's method 16.

## BEST MODE FOR CARRYING OUT THE INVENTION

Hereinafter, the reasons are described for restricting the chemical composition and the texture of a rare earth magnet powder of the present invention, as well as for restricting the production condition and the addition amount of a Dy hydride powder, a Tb hydride powder, or a Dy—Tb binary alloy hydride powder added to a rare earth magnet alloy raw material powder or a hydrogen-absorbing rare earth magnet alloy raw material powder in a method of producing a rare earth magnet powder which is excellent in magnetic anisotropy and thermal stability of the present invention, as described above.

## (A) Rare Earth Magnet Powder

## (i) Reasons for Restricting Chemical Compositions

R:

R is a rare earth element which primarily includes Nd and also includes small amounts of, for example, Y, Pr, Sm, Ce, La, Er, Eu, Gd, Tm, Yb, Lu, and Ho (but excludes Dy and Tb). When the content of R is less than 5%, coercivity decreases, while when the content of R is more than 20%, saturation magnetization decreases; thus, the desired magnetic properties cannot be achieved in either of these cases. Therefore, the content of R has been set at 5 to 20%.

## Dy and Tb:

The content of one or both of Dy and Tb has been set at 0.01 to 10% (particularly preferably 0.3 to 4%). The reasons thereof are as follows. When the content of one or both of Dy and Tb is less than 0.01%, the desired effects of the present invention that is excellent magnetic anisotropy and thermal stability cannot be obtained, while when the content of one or both of Dy and Tb is more than 10%, anisotropy 5 decreases and appropriate magnetic properties cannot be obtained.

B:

When the content of B is less than 3%, coercivity decreases, while when the content of B is more than 20%, saturation magnetization decreases; thus, the desired mag-

## 12

netic properties cannot be achieved in either of these cases. Therefore, the content 10 of B has been set at 3 to 20%.

Co:

Co is optionally added to prevent the rare earth magnet alloy from changing to an isotropic state. When the content of Co is less than 0.1%, the desired effect cannot be obtained, while when the content of Co is more than 50%, coercivity and saturation magnetization decreases, so high properties cannot be obtained even if the rare earth magnet alloy becomes in an anisotropic state. Therefore, the content of Co has been set at 0.1 to 50% (particularly preferably 5 to 30%), which is contained in a rare earth magnet powder of the present invention and a rare earth magnet alloy raw material used in a method of producing a rare earth magnet powder of the present invention.

M (One, or Two or More from Among Ga, Zr, Nb, Mo, Hf, Ta, W, Ni, Al, Ti, V, Cu, Cr, Ge, C and Si):

M is optionally added to furter improve coercivity and remanence. When the content of M is less than 0.001%, the desired effect cannot be obtained, while when the content of M is more than 5%, the coercivity and the remanence decrease. Therefore, the content of M has been set at 0.001 to 5%.

## (ii) Reasons for Restricting Textures

## Maximum Detected Intensity in Line Analysis by Using Wavelength Dispersive X-ray Spectroscopy:

The maximum detected intensity of one or both of Dy and Tb near the surface can be obtained as follows: scanning across a powder cross-section in line analysis by using wavelength dispersive X-ray spectroscopy; obtaining the average detected intensity in the central portion being present in the range of  $\frac{1}{3}$  of the particle diameter of a powder particle and referring to this as a near-center intensity; and determining the maximum detected intensity of one or both of Dy and Tb at a peak near the surface as a ratio relative to the near-center intensity. Herein, the place sometimes appears where the detected intensity of one or both of Dy and Tb is locally very large, while this is usually due to the presence of a rare earth rich phase, and it is a characteristic of this phase that, in addition to one or both of Dy and Tb, the detected intensity of one or both of Nd and Pr also increases at the same time. Because such a phase inevitably occurs in the present invention, it shall be excluded from assessments of the maximum detected intensity. Also, when the maximum detected intensity of one or both of Dy and Tb by using wavelength dispersive X-ray spectroscopy here is less than 1.2 times the near-center intensity, because of the small anisotropic magnetic field difference between the surface and the interior of a powder particle, the desired effect of achieving both large coercivity due to a highly anisotropic magnetic field at the surface and large anisotropy at the interior cannot be obtained. Also, when the detected intensity is more than 5 times the near-center intensity, magnetic flux density in the near-surface region decreases remarkably. Therefore, the detected intensity of one or both of Dy and Tb in the near-surface region by using wavelength dispersive X-ray spectroscopy has been set at 1.2 to 5 times (preferably 1.3 to 4 times) the detected intensity at the interior.

## Thickness of Dy—Tb Rich Layer from Surface:

The depth, from the surface, of the region being rich in content of one or both of Dy and Tb (Dy—Tb rich layer) which is present at the surface of the rare earth magnet powder can be obtained as follows: scanning across the vicinity of the surface in a powder cross-section at as fine intervals as pos-

sible in line analysis by using wavelength dispersive X-ray spectroscopy; and determining the width of a portion in which the detected intensity of a peak is at least 1.2 times the average detected intensity near the center as the depth of the region of the region being rich in content of one or both of Dy and Tb from the surface. Herein, when a Dy—Tb rich phase in which a detected intensity of one or both of Dy and Tb is locally very high exists in the scanned area, this area is excluded from assessment of the depth from the surface. It is believed that, in a Dy—Tb rich layer, one or both of Dy and Tb substitutes for an R atom of a  $R_2(Fe,Co)_{14}B$  crystal grain near the surface so as to form a  $(R,(Dy,Tb))_2(Fe,Co)_{14}B$  phase and that the effects of the present invention are obtained by the substitution resulting in one or more layer of crystal grains at the surface having more one or both of Dy and Tb than at the interior of a particle. However, the desired effects are not obtained when the Dy—Tb rich layer which is the region being rich in content of one or both of Dy and Tb has a thickness of less than 0.05  $\mu m$ . On the other hand, when the Dy—Tb rich layer has a thickness of more than 50  $\mu m$ , the volume of the region having the high content of one or both of Dy and Tb and large coercivity has an influence on the highly anisotropic region at the interior, so as to remarkably lower the anisotropy of the powder as a whole. Accordingly, the depth of the Dy—Tb rich layer from the surface has been set at 0.05 to 50  $\mu m$  (preferably 1 to 30  $\mu m$ ).

#### Surface Coverage of Dy—Tb Rich Layer:

The surface coverage of the region being rich in content of one or both of Dy and Tb (Dy—Tb rich layer) is obtained as follows: carrying out five or more line analyses at different scanning positions on a single powder cross-section in line analysis by wavelength dispersive X-ray spectroscopy; and determining the surface coverage of a Dy—Tb rich layer as the ratio of the number of powder surfaces, for which the sum of the detected intensity of one or both of Dy and Tb near the surface of the powder is at least 1.2 times that near the center, to the number of times the powder surfaces were crossed by scanning. Herein, when a rare earth rich phase in which a detected intensity of one or both of Dy and Tb is locally very high exists in the scanned area, this area is excluded from the count. The surface of the powder is covered by the region having a strong anisotropic magnetic field and being rich in content of one or both of Dy and Tb which are elements being less readily oxidized than Nd, so the powder has large coercivity and large anisotropy, and excellent resistance to oxidation can be obtained. However, when less than 70% of the surface is covered by the region, sufficiently large coercivity cannot be obtained, and the resistance to oxidation is also insufficient, so sufficient thermal stability and heat resistance cannot be obtained. Accordingly, the surface area covered by the region being rich in content of one or both of Dy and Tb has been set at 70% or more (preferably 80% or more) of the entire surface of the powder.

In the rare earth magnet powder of the present invention, it is believed that the coercivity of the powder is improved because the region being rich in content of one or both of Dy and Tb (Dy—Tb rich layer) near the surface at the powder interior has a higher anisotropic magnetic field than vicinity of the center. Moreover, it is believed that the thermal stability and the heat resistance of the powder are improved because Dy and Tb are relatively resistant to oxidation and improve the resistance to oxidation of the powder. In addition, it is believed that the anisotropy of the powder as a whole rarely decreases because the region being rich in content of one or both of Dy and Tb (Dy—Tb rich layer) is restricted to the

vicinity of the powder surface. This is most likely why the powder exhibits both good heat resistance and high anisotropy.

#### (B) Reasons for Restricting the Production Conditions in the Methods of Producing a Rare Earth Magnet Powder which is Excellent in Magnetic Anisotropy and Thermal Stability Described in Any One of the Aforementioned (7) to (11):

The reasons for milling the rare earth magnet alloy raw material to an average particle diameter of 10 to 1,000  $\mu m$  (preferably 50 to 400  $\mu m$ ) are as follows. When fine milling to an average particle diameter of below 10  $\mu m$  is attempted in an inert gas atmosphere, the oxidation of the alloy due to heat generation during milling is unavoidable because of the very small particle diameter, whereby the coercivity of the rare earth magnet powder ultimately obtained is unfavorably lowered. On the other hand, when an average particle diameter is longer than 1,000  $\mu m$ , Dy, Tb, or a Dy—Tb binary alloy is not able to diffuse to the center portion of the rare earth magnet alloy raw material powder, resulting in an inhomogeneous composition. Then, the axis of easy magnetization in each particle of the rare earth magnet powder ultimately obtained by pulverizing is difficult to align, so the magnetic anisotropy is unfavorably lowered.

A rare earth magnet powder which is further excellent magnetic anisotropy and thermal stability can be obtained by the following method including: adding to the aforementioned rare earth magnet alloy raw material powder a Dy hydride powder, a Tb hydride powder, or a Dy—Tb binary alloy hydride powder, each of which has an average powder particle diameter of 0.1 to 50  $\mu m$ , at 0.01 to 5 mol %, followed by mixing so as to produce a mixed powder; carrying out hydrogen absorption by heating, or heating and holding the mixed powder from room temperature to a temperature below 500° C. in a hydrogen gas atmosphere with a pressure of 10 to 1,000 kPa so as to induce the mixed powder to absorb hydrogen; carrying out hydrogen absorption-decomposition by heating and holding the mixed powder at a temperature in a range of 500 to 1,000° C. in a hydrogen gas atmosphere with a pressure of 10 to 1,000 kPa so as to induce the mixed powder to absorb hydrogen and to be decomposed; and then carrying out hydrogen desorption by holding the mixed powder at a temperature in a range of 500 to 1,000° C. in a vacuum atmosphere with an ultimate pressure of 0.13 kPa or below so as to forcibly release hydrogen and promote a phase transformation, followed by cooling and pulverizing.

When the mixed powder obtained by adding to the aforementioned rare earth magnet alloy raw material powder a Dy hydride powder, a Tb hydride powder or a Dy—Tb binary alloy hydride powder, followed by mixing, is subjected to hydrogen absorption; hydrogen absorption-decomposition; and then hydrogen desorption, a rare earth magnet powder which is further excellent in magnetic anisotropy and thermal stability is obtained. The following reasons are believed for this.

It has been found from recent research that the reactions at the stage of hydrogen absorption-decomposition are important in the case of anisotropizing a rare earth magnet powder by subjecting a rare earth magnet alloy raw material powder to the treatment including, in turn, hydrogen absorption, hydrogen absorption-decomposition, and then hydrogen desorption (which is generally referred to as HDDR treatment). On the other hand, when a large amount of one or both of Dy and Tb is added to the rare earth magnet alloy in an attempt to increase coercivity for the purpose of the thermal stability, as described in Patent document (Japanese Patent Application, First Publication No. 1997-165601), anisotropy decreases,

and a sufficient energy product cannot be obtained. This is probably because the inclusion of a large amount of one or both of Dy and Tb in the rare earth magnet alloy affects the reactions of the aforementioned hydrogen absorption-decomposition; therefore, the state formed by the hydrogen absorption-decomposition reactions does not satisfy the conditions for anisotropization.

However, when the mixed powder, which is produced by adding a Dy hydride powder, a Tb hydride powder, or a Dy—Tb binary alloy hydride powder to the rare earth magnet alloy raw material powder obtained by milling in an ordinary inert gas atmosphere, followed by mixing, is subjected to the hydrogen absorption-decomposition as in the present invention, the decomposition reactions at that time proceed toward the formation of rare earth element hydrides formed from the rare earth magnet alloy and the decomposition of the residue into the phase primarily including Fe or (Fe,Co), and Fe<sub>2</sub>B. Because a Dy hydride powder, a Tb hydride powder, or a Dy—Tb binary alloy hydride powder, which is a rare earth element, does not take part in these decomposition reactions, only the rare earth magnet alloy raw material powder is decomposed. Therefore, unlike when a large amount of one or both of Dy and Tb is added to a rare earth magnet alloy, the state formed by the hydrogen absorption-decomposition reactions does not fail to satisfy the conditions for anisotropization.

Subsequently, when hydrogen desorption is carried out from the aforementioned state, the phase primarily including R hydrides, Fe or (Fe,Co), and Fe<sub>2</sub>B, which have been decomposed in the rare earth magnet alloy raw material powder, reacts so as to form a R<sub>2</sub>Fe<sub>14</sub>B-based phase. In addition, a Dy hydride powder, a Tb hydride powder, or a Dy—Tb binary alloy hydride powder also releases hydrogen, so one or both atoms of Dy and Tb diffuse in the entire surface of the rare earth magnet alloy raw material powder, and then diffuse into the interior of the rare earth magnet alloy raw material powder. Therefore, the R<sub>2</sub>Fe<sub>14</sub>B-based phase that is ultimately formed has a higher content of one or both of Dy and Tb than the original rare earth magnet alloy raw material powder, and the content of one or both of Dy and Tb near the surface in each powder particle is higher than the content near the center therein. As a result, coercivity is improved, and the temperature coefficient of coercivity decreases, thereby improving the thermal stability. Meanwhile, the following reason can also be believed. The conditions for anisotropization are satisfied at the stage of the hydrogen absorption-decomposition reactions, so anisotropization in fact occurs due to the hydrogen desorption, thereby providing a rare earth magnet powder which is excellent in coercivity and anisotropy.

In the present invention, by adding to the aforementioned rare earth magnet alloy raw material powder a Dy hydride powder, a Tb hydride powder, or a Dy—Tb binary alloy hydride powder, each of which has an average powder particle diameter of 0.1 to 50 µm, at 0.01 to 5 mol %, followed by mixing so as to produce a mixed powder; heating the mixed powder further; and then carrying out hydrogen absorption-decomposition by heating and holding the mixed powder at a predetermined temperature in a range of 500 to 1,000° C. in a hydrogen gas atmosphere with a pressure of 10 to 1,000 kPa, the raw material is induced to absorb hydrogen, thereby promoting a phase transformation and causing decomposition to occur. A Dy hydride powder, a Tb hydride powder, or a Dy—Tb binary alloy hydride powder, which is added to the rare earth magnet alloy raw material powder so as to produce the mixed powder, is restricted to have an average particle diameter in a range of 0.1 to 50 µm for the following reasons.

When a Dy hydride powder, a Tb hydride powder, or a Dy—Tb binary alloy hydride powder has an average particle diameter of less than 0.1 µm, intense oxidation occurs, thereby making the powder very difficult to handle. On the other hand, when a Dy hydride powder, a Tb hydride powder, or a Dy—Tb binary alloy hydride powder has an average particle diameter of more than 50 µm, a phase of Dy, Tb, or a Dy—Tb binary alloy, or a compound phase having an excess of these elements segregates in the rare earth magnet powder, so it is impossible to diffuse uniformly. Therefore, the average particle diameter of these hydride powders has been set at 0.1 to 50 µm (more preferably 1 to 10 µm).

Also, the addition amount of a Dy hydride powder, a Tb hydride powder, or a Dy—Tb binary alloy hydride powder is restricted to be 0.01 to 5 mol % for the following reasons. At less than 0.01 mol %, a coercivity-improving effect cannot be obtained sufficiently. On the other hand, the addition of more than 5 mol % lowers the anisotropy, so sufficient magnetic properties cannot be obtained. Therefore, the addition amount of a Dy hydride powder, a Tb hydride powder, or a Dy—Tb binary alloy hydride powder was set at 0.01 to 5 mol % (more preferably 0.3 to 3 mol %).

The conditions under which the temperature is raised, or raised and held, from room temperature to a temperature below 500° C. in a hydrogen gas atmosphere with a pressure of 10 to 1,000 kPa during the hydrogen absorption treatment are already known. Likewise, the conditions under which the mixed powder is held at a predetermined temperature in a range of 500 to 1,000° C. in a hydrogen gas atmosphere with a pressure of 10 to 1,000 kPa during the subsequent hydrogen absorption-decomposition treatment are also already known. Because neither are particularly novel conditions, an explanation of the reasons for these limits is omitted here.

Following such hydrogen absorption-decomposition, intermediate heat treatment is carried out if necessary. This intermediate heat treatment is a step that accelerates anisotropization at a suitable speed by using an inert gas flow to change the atmosphere to an inert gas atmosphere. This intermediate heat treatment is carried out under conditions of holding the powder at a predetermined temperature in a range of 500 to 1,000° C. in an inert gas atmosphere with a pressure of 10 to 1,000 kPa. When an inert gas atmosphere pressure during the intermediate heat treatment is less than 10 kPa, anisotropization is unfavorably too rapid, causing a decrease of coercivity. On the other hand, when an inert gas atmosphere pressure during the intermediate heat treatment is more than 1,000 kPa, anisotropization substantially does not proceed, causing an unfavorable decrease of remanence.

Following the optional intermediate heat treatment, heat treatment in depressurized hydrogen is carried out if necessary. This heat treatment in depressurized hydrogen is a step in which the mixed powder subjected to hydrogen absorption-decomposition is held in a hydrogen atmosphere with an absolute pressure of at least 0.65 but less than 10 kPa (preferably 2 to 8 kPa) or in a mixed hydrogen/inert gas atmosphere with a hydrogen partial pressure of at least 0.65 but less than 10 kPa (preferably 2 to 8 kPa) so as to heat-treat the mixed powder with some hydrogen remaining therein. By carrying out this heat treatment in depressurized hydrogen, coercivity and remanence can be further improved.

After carrying out the optional intermediate heat treatment and the heat treatment in depressurized hydrogen, hydrogen desorption is carried out. Hydrogen desorption is a treatment holding the mixed powder in a vacuum atmosphere with an ultimate pressure of 0.13 kPa or below so as to forcibly release sufficient hydrogen from the mixed powder, thereby further promoting a phase transformation. The mixed powder

is held in a vacuum atmosphere with an ultimate pressure of 0.13 kPa or less because sufficient hydrogen desorption is not carried out at an ultimate pressure exceeding 0.13 kPa.

In cooling carried out following the hydrogen desorption, the mixed powder is cooled to room temperature by flowing inert gas (Ar gas). Cooling is followed by pulverizing so as to produce a rare earth magnet powder. The rare earth magnet powder thus obtained by pulverizing has very low residual internal stress, and so does not require heat treatment. By binding the rare earth magnet powder obtained by the production method of the invention, which is further excellent in magnetic anisotropy and thermal stability, with an organic binder or metal binder, a rare earth magnet which is excellent in magnetic anisotropy and thermal stability can be produced. Alternatively, by molding this rare earth magnet powder, a green compact can be produced, and by processing the green compact with hot pressing or hot isostatic pressing at a temperature of 600 to 900° C., a rare earth magnet which is excellent in magnetic anisotropy and thermal stability can be produced.

(C) Reasons for Restricting Production Conditions in the Methods of Producing a Rare Earth Magnet Powder which is Excellent in Magnetic Anisotropy and Thermal Stability Described in Any One of the Aforementioned (12) to (16):

The hydrogen-absorbing rare earth magnet alloy raw material powder is produced by subjecting the rare earth magnet alloy raw material to the hydrogen absorption by heating the rare earth magnet alloy raw material from room temperature to a predetermined temperature below 500° C., or heating and holding at a predetermined temperature below 500° C. (for example, 100° C.), in a hydrogen gas atmosphere with a pressure of 10 to 1,000 kPa so as to induce the rare earth magnet alloy raw material to absorb hydrogen. This hydrogen absorption of heating the rare earth magnet alloy raw material from room temperature to a predetermined temperature below 500° C., or heating and holding at a predetermined temperature below 500° C. (for example, 100° C.), in a hydrogen gas atmosphere with a pressure of 10 to 1,000 kPa is a treatment that is carried out conventionally. In the present invention, the reasons for producing a hydrogen-absorbing rare earth magnet alloy raw material powder by milling this rare earth magnet alloy raw material subjected to the hydrogen absorption are the following.

A bulk rare earth magnet alloy raw material subjected to the hydrogen absorption is easy to mill.

The material is easier to mill than when milling is carried out in another step where the material is held at a high temperature because the hydrogen absorption is carried out at a relatively low temperature below 500° C.

A sufficiently fine rare earth magnet powder can be obtained merely by pulverization in a final milling step because the bulk rare earth magnet alloy raw material is subjected to the hydrogen absorption, then milled beforehand to about the same average particle diameter as the rare earth magnet powder. Therefore, oxidation of the obtained rare earth magnet powder very rarely occurs and internal stresses very rarely build up, thereby further improving the magnetic anisotropy.

When HDDR treatment is carried out following hydrogen pulverization, the surface unevenness of the magnet powder decreases, resulting in a smooth surface, and the specific surface area decreases, thereby improving thermal stability.

In the production of the hydrogen-absorbing rare earth magnet alloy raw material, the reason for milling the rare earth magnet alloy raw material to an average powder particle

diameter of 10 to 1,000 μm (more preferably 50 to 400 μm) following the hydrogen absorption is as follows. Bulk rare earth magnet alloy raw material subjected to the hydrogen absorption is relatively resistant to oxidation, but when fine milling to an average particle diameter below 10 μm is attempted, the very small diameter makes oxidation inevitable during milling, and such oxidation has the undesirable effect of lowering the coercivity of the rare earth magnet powder ultimately obtained. On the other hand, when an average particle diameter is longer than 1,000 μm, the axis of easy magnetization in each powder particle of the rare earth magnet powder ultimately obtained by pulverizing is difficult to align, so the magnetic anisotropy is lowered unfavorably. The hydrogen-absorbing rare earth magnet alloy raw material powder has substantially the same average particle diameter as the rare earth magnet powder ultimately obtained.

A rare earth magnet powder which is excellent in magnetic anisotropy and thermal stability can be obtained by adding to the aforementioned hydrogen-absorbing rare earth magnet alloy raw material powder a Dy hydride powder, a Tb hydride powder, or a Dy—Tb binary alloy hydride powder, each of which has an average powder particle diameter of 0.1 to 50 μm, at 0.01 to 5 mol %, followed by mixing so as to produce a hydrogen-containing raw material mixed powder; carrying out hydrogen absorption-decomposition by heating and holding the hydrogen-containing raw material mixed powder at a temperature in a range of 500 to 1,000° C. in a hydrogen gas atmosphere with a pressure of 10 to 1,000 kPa so as to induce the hydrogen-containing raw material mixed powder to absorb further hydrogen and to be decomposed; and then carrying out hydrogen desorption by holding the hydrogen-containing raw material mixed powder at a temperature in a range of 500 to 1,000° C. in a vacuum atmosphere with an ultimate pressure of 0.13 kPa or below so as to forcibly release hydrogen and promote a phase transformation, followed by cooling and pulverizing.

When the hydrogen-containing mixed powder, which is obtained by adding to the hydrogen-absorbing rare earth magnet alloy raw material powder a Dy hydride powder, a Tb hydride powder or a Dy—Tb binary alloy hydride powder, followed by mixing, is subjected to hydrogen absorption-decomposition followed by hydrogen desorption, a rare earth magnet powder which is further excellent in magnetic anisotropy and thermal stability is obtained. The reasons are as follows.

It has been found from recent research that the reactions at the stage of hydrogen absorption-decomposition are important in the case of anisotropizing a rare earth magnet powder by carrying out the HDDR treatment. On the other hand, when a large amount of one or both of Dy and Tb is added to the rare earth magnet alloy in an attempt to increase the coercivity for the purpose of the thermal stability, as described in Patent document (Japanese Patent Application, First Publication No. 1997-165601), the anisotropy decreases, and a sufficient energy product cannot be obtained. This is probably because the inclusion of a large amount of one or both of Dy and Tb in the rare earth magnet alloy affects the reactions of the aforementioned hydrogen absorption-decomposition; therefore, the state formed by the hydrogen absorption-decomposition reactions does not satisfy the conditions for anisotropization.

However, when the hydrogen-containing raw material mixed powder, which is produced by adding a Dy hydride powder, a Tb hydride powder, or a Dy—Tb binary alloy hydride powder to the rare earth magnet alloy raw material powder subjected to the hydrogen absorption, followed by mixing, is subjected to the hydrogen absorption-decomposi-

tion as in the present invention, the decomposition reactions at that time proceed toward the formation of rare earth element hydrides formed from the rare earth magnet alloy and the decomposition of the residue into the phase primarily including Fe or (Fe,Co), and Fe<sub>2</sub>B. Because a Dy hydride powder, a Tb hydride powder, or a Dy—Tb binary alloy hydride powder, which is a rare earth element, does not take part in these decomposition reactions, only the rare earth magnet alloy raw material powder is decomposed. Therefore, unlike when a large amount of one or both of Dy and Tb is added to a rare earth magnet alloy, the state formed by the hydrogen absorption-decomposition reactions does not fail to satisfy the conditions for anisotropization.

Subsequently, when hydrogen desorption is carried out from the aforementioned state, the phase primarily including R hydrides, Fe or (Fe,Co), and Fe<sub>2</sub>B, which have been decomposed in the rare earth magnet alloy raw material powder, reacts so as to form a R<sub>2</sub>Fe<sub>14</sub>B-based phase. In addition, a Dy hydride powder, a Tb hydride powder, or a Dy—Tb binary alloy hydride powder also releases hydrogen, so one or both atoms of Dy and Tb diffuse in the entire surface of the rare earth magnet alloy raw material powder, and then diffuse into the interior of the rare earth magnet alloy raw material powder. Therefore, the R<sub>2</sub>Fe<sub>14</sub>B-based phase that is ultimately formed has a higher content of one or both of Dy and Tb than the original rare earth magnet alloy raw material powder, and the content of one or both of Dy and Tb near the surface in each powder particle is higher than the content near the center therein. As a result, coercivity is improved, and the temperature coefficient of coercivity decreases, thereby improving the thermal stability. Meanwhile, the following reason can also be believed. The conditions for anisotropization are satisfied at the stage of the hydrogen absorption-decomposition reactions, so anisotropization in fact occurs due to the hydrogen desorption, thereby providing a rare earth magnet powder which is excellent in coercivity and anisotropy.

In the present invention, by adding to the aforementioned hydrogen-absorbing rare earth magnet alloy raw material powder a Dy hydride powder, a Tb hydride powder, or a Dy—Tb binary alloy hydride powder, each of which has an average powder particle diameter of 0.1 to 50 µm, at 0.01 to 5 mol %, followed by mixing so as to produce a hydrogen-containing raw material mixed powder; heating the hydrogen-containing raw material mixed powder further; and then carrying out hydrogen absorption-decomposition by heating and holding the mixed powder at a predetermined temperature in a range of 500 to 1,000° C. in a hydrogen gas atmosphere with a pressure of 10 to 1,000 kPa, the raw material is induced to absorb hydrogen, thereby promoting a phase transformation and causing decomposition to occur.

A Dy hydride powder, a Tb hydride powder, or a Dy—Tb binary alloy hydride powder, which is added to the hydrogen-absorbing rare earth magnet alloy raw material powder so as to produce the hydrogen-containing raw material mixed powder, is restricted to have an average particle diameter in a range of 0.1 to 50 µm for the following reasons. When a Dy hydride powder, a Tb hydride powder, or a Dy—Tb binary alloy hydride powder has an average particle diameter of less than 0.1 µm, intense oxidation occurs, thereby making the powder very difficult to handle. On the other hand, when a Dy hydride powder, a Tb hydride powder, or a Dy—Tb binary alloy hydride powder has an average particle diameter of more than 50 µm, a phase of Dy, Tb, or a Dy—Tb binary alloy, or a compound phase having an excess of these elements segregates in the rare earth magnet powder, so it is impossible to diffuse uniformly. Therefore, the average particle diameter of these hydride powders has been set at 0.1 to 50 µm (more

preferably 1 to 10 µm). Also, the addition amount of a Dy hydride powder, a Tb hydride powder, or a Dy—Tb binary alloy hydride powder is restricted to be 0.01 to 5 mol % for the following reasons. At less than 0.1 mol %, a coercivity-improving effect cannot be obtained sufficiently. On the other hand, the addition of more than 5 mol % lowers the anisotropy, so sufficient magnetic properties cannot be obtained. Therefore, the addition amount of a Dy hydride powder, a Tb hydride powder, or a Dy—Tb binary alloy hydride powder was set at 0.01 to 5 mol % (more preferably 0.3 to 3 mol %).

The conditions under which the hydrogen-containing raw material mixed powder is held at a predetermined temperature in a range of 500 to 1,000° C. in a hydrogen gas atmosphere with a pressure of 10 to 1,000 kPa during the subsequent hydrogen absorption-decomposition treatment are already known. Because they are not particularly novel conditions, an explanation of the reasons for these limits is omitted here.

Following such hydrogen absorption-decomposition, intermediate heat treatment is carried out if necessary. This intermediate heat treatment is a step that accelerates anisotropization at a suitable speed by using an inert gas flow to change the atmosphere to an inert gas atmosphere. This intermediate heat treatment is carried out under conditions of holding the powder at a predetermined temperature in a range of 500 to 1,000° C. in an inert gas atmosphere having a pressure of 10 to 1,000 kPa. When an inert gas atmosphere pressure during the intermediate heat treatment is less than 10 kPa, anisotropization is unfavorably too rapid, causing a decrease of the coercivity. On the other hand, at more than 1,000 kPa, anisotropization substantially does not proceed, causing an unfavorable decrease of the remanence.

Following the optional intermediate heat treatment, heat treatment in depressurized hydrogen is carried out if necessary. This heat treatment in depressurized hydrogen is a step in which the hydrogen-containing raw material mixed powder subjected to hydrogen absorption-decomposition is held in a hydrogen atmosphere with an absolute pressure of at least 0.65 but less than 10 kPa (preferably 2 to 8 kPa) or in a mixed hydrogen/inert gas atmosphere with a hydrogen partial pressure of at least 0.65 but less than 10 kPa (preferably 2 to 8 kPa) so as to heat-treat the hydrogen-containing raw material mixed powder with some hydrogen remaining therein. By carrying out this heat treatment in depressurized hydrogen, coercivity and remanence can be further improved.

After carrying out the optional intermediate heat treatment and heat treatment in depressurized hydrogen, hydrogen desorption is carried out. Hydrogen desorption is a treatment holding the hydrogen-containing raw material mixed powder in a vacuum atmosphere with an ultimate pressure of 0.13 kPa or below so as to forcibly release sufficient hydrogen from the hydrogen-containing raw material mixed powder, thereby further promoting a phase transformation. The hydrogen-containing raw material mixed powder is held in a vacuum atmosphere with an ultimate pressure of 0.13 kPa or less because sufficient hydrogen desorption is not carried out at an ultimate pressure exceeding 0.13 kPa.

In cooling carried out following the hydrogen desorption, the hydrogen-containing raw material mixed powder is cooled to room temperature by flowing inert gas (Ar gas). Cooling is followed by pulverizing so as to produce a rare earth magnet powder. The rare earth magnet powder thus obtained by pulverizing has very low residual internal stress, and so does not require heat treatment. By binding the rare earth magnet powder obtained by the production method of the invention, which is further excellent in magnetic anisotropy and thermal stability, with an organic binder or metal

binder, a rare earth magnet which is excellent in magnetic anisotropy and thermal stability can be produced. Alternatively, by molding this rare earth magnet powder, a green compact can be produced, and by processing the green compact with hot pressing or hot isostatic pressing at a temperature of 600 to 900°C., a rare earth magnet which is excellent in magnetic anisotropy and thermal stability can be produced.

The rare earth magnet alloy raw material, which is used in the method of producing a rare earth magnet powder which is excellent in magnetic anisotropy and thermal stability described in any one of the aforementioned (7) to (16), may or may not include one or both of Dy and Tb. Therefore, the rare earth magnet alloy raw material, which is used in the method of producing a rare earth magnet powder which is excellent in magnetic anisotropy and thermal stability of the present invention, has the same chemical composition as the rare earth magnet alloy raw materials used to produce the conventional magnetically anisotropic HDDR magnet powders described in Patent documents 1 and 2. More specifically, when one, or two or more rare earth elements which includes Y, and may or may not include one or both of Dy and Tb is referred to as R', the rare earth magnet alloy raw material in the present invention includes:

a chemical composition including R': 10 to 20% and B: 3 to 20%, with the balance including Fe and inevitable impurities;

a chemical composition including R': 10 to 20%, B: 3 to 20%, and M: 0.001 to 5%, with the balance including Fe and inevitable impurities;

a chemical composition including R': 10 to 20%, Co: 0.1 to 50%, and B: 3 to 20%, with the balance including Fe and inevitable impurities; or

a chemical composition including R': 10 to 20%, Co: 0.1 to 50%, B: 3 to 20%, and M: 0.001 to 5%, with the balance including Fe and inevitable impurities.

## EXAMPLES

Hereinafter, examples of the present invention are described, while the present invention is not restricted to these examples.

Ingots a to o of rare earth magnet alloy raw materials having the chemical compositions shown in Table 1 were produced by melting the respective raw materials in a high-frequency vacuum melting furnace, casting the obtained melts, and carrying out homogenizing treatment by holding the ingots at 1,100°C. for 24 hours in an Ar gas atmosphere. These ingots a to o were crushed in an Ar gas atmosphere so as to produce blocks up to 10 mm in size.

TABLE 1

| Type  | Chemical composition (in atom %) (wherein balance: Fe)                |
|-------|-----------------------------------------------------------------------|
| Ingot |                                                                       |
| a     | Nd: 12.3%, Co: 17.0%, B: 6.5%, Zr: 0.1%, Ga: 0.3%                     |
| b     | Nd: 11.6%, Dy: 1.8%, Pr: 0.2%, B: 6.1%                                |
| c     | Nd: 11.5%, Dy: 0.8%, Pr: 0.2%, Co: 7.0%, B: 6.5%, Zr: 0.1%, Ti: 0.3%  |
| d     | Nd: 12.5%, Pr: 0.5%, Co: 18.0%, B: 6.5%, Zr: 0.1%, Ga: 0.3%           |
| e     | Nd: 11.9%, La: 0.4%, Co: 14.7%, B: 6.8%, Hf: 0.1%, Si: 0.3%, W: 0.5%  |
| f     | Nd: 12.0%, Dy: 2.0%, B: 6.5%, Hf: 0.1%                                |
| g     | Nd: 12.3%, Dy: 1.8%, Co: 16.9%, B: 6.6%, Zr: 0.2%, Ga: 0.3%, Al: 0.5% |
| h     | Nd: 11.0%, Pr: 3.0%, Co: 20.0%, B: 6.5%, Si: 0.1%, Ga: 0.3%           |
| i     | Nd: 9.0%, Ce: 4.0%, Co: 10.0%, B: 6.5%, Nb: 0.4%                      |
| j     | Nd: 8.0%, Dy: 5.0%, Co: 5.0%, B: 6.5%, Zr: 0.1%, Ta: 0.4%             |
| k     | Nd: 11.4%, Dy: 2.1%, Co: 15.0%, B: 7.0%                               |

TABLE 1-continued

| Type | Chemical composition (in atom %) (wherein balance: Fe)               |
|------|----------------------------------------------------------------------|
| l    | Nd: 12.2%, Tb: 1.2%, Co: 12.0%, B: 7.5%, Ge: 0.3%, Cr: 0.1%          |
| m    | Nd: 11.3%, Pr: 2.0%, Gd: 1.0%, B: 6.8%, V: 0.3%, Cu: 0.1%            |
| n    | Nd: 12.4%, Dy: 1.0%, Co: 8.0%, B: 6.5%, Ni: 0.1%, Mo: 0.3%           |
| o    | Nd: 11.2%, Pr: 2.0%, Co: 11.2%, B: 6.5%, Zr: 0.1%, Ga: 0.3%, C: 0.2% |

## Example 1

The present invention's methods 1 to 5 were carried out as follows. Blocks obtained from ingots a to e in Table 1 were milled in an Ar gas atmosphere to the average particle diameters shown in Table 2 so as to produce rare earth magnet alloy raw material powders. To these rare earth magnet alloy raw material powders, a Dy hydride powder, a Tb hydride powder, or a Dy—Tb binary alloy hydride powder, each of which has an average particle diameter of 5 µm was added thereto at the amount shown in Table 2, and then mixed therewith so as to produce mixed powders. The respective mixed powders were then subjected to, in order, hydrogen absorption under the conditions shown in Table 2; hydrogen absorption-decomposition under the conditions shown in Table 2; if necessary, intermediate heat treatment under the conditions shown in Table 2; if necessary, heat treatment in depressurized hydrogen under the conditions shown in Table 2; hydrogen desorption under the conditions shown in Table 3; forcibly cooling to room temperature with Ar gas; and then pulverizing to 300 µm or below, thereby producing rare earth magnet powders.

## Conventional Example 1

Conventional methods 1 to 5 were carried out as follows. Blocks obtained from ingots a to e in Table 1 were subjected to hydrogen absorption under the same conditions as in Example 1 and shown in Table 2 without milling the blocks nor adding a hydride powder so as to produce a mixed powder, and then were subjected to, in order, hydrogen absorption-decomposition under the same conditions as in Example 1 and shown in Table 2; if necessary, heat treatment in depressurized hydrogen under the conditions shown in Table 2; forcibly cooling to room temperature in Ar gas; and then milling treatment to the average particle diameter shown in Table 3 so as to produce rare earth magnet raw material hydride powders. Then, to these rare earth magnet raw material hydride powders, a Dy hydride powder, a Tb hydride powder, or a Dy—Tb binary alloy hydride powder, each of which has an average particle diameter of 5 µm, was added at the amount shown in Table 3 and then mixed therewith so as to produce hydrogen-containing raw material mixed powders. Each of these hydrogen-containing raw material mixed powders was subjected to diffusion heat-treating including heating in a vacuum followed by holding under the conditions shown in Table 3; hydrogen desorption under the conditions shown in Table 3; forcibly cooling to room temperature with Ar gas; and then pulverizing to 300 µm or below, thereby producing rare earth magnet powders.

Each of the rare earth magnet powders obtained by using the present invention's methods 1 to 5 and the conventional methods 1 to 5 was embedded in a phenolic resin and polished to a mirror surface, and the detected intensities of near-center and near-surface Dy and/or Tb and the intensity ratio thereof

were measured by analysis with an electron probe microanalyzer (hereinafter abbreviated as "EPMA"; model JXA-8800RL manufactured by JEOL Ltd.) which is a type of wavelength dispersive X-ray spectrometer, thereby determining the values of the depth of the Dy—Tb rich layer from the surface and of the surface coverage by the Dy—Tb rich layer. Those results are given in Table 4.

In addition, to each of the rare earth magnet powders obtained in the present invention's methods 1 to 5 and the conventional methods 1 to 5, an epoxy resin was added at 3 wt % and then mixed therewith, and each of the mixtures was compression-molded in a magnetic field of 1.6 MA/m so as to produce a green compact. The green compact was hardened in an oven at 150° C. for 2 hours so as to produce a bonded magnet having a density of 6.0 to 6.1 g/cm<sup>3</sup>. The magnetic properties of the obtained bonded magnet are shown in Table 5. Also, the temperature coefficient of coercivity  $\alpha_{iHc}$  for each magnet was determined from the result of the magnetic properties measured at 150° C., and those values are shown in Table 5. Herein, the temperature coefficient of coercivity  $\alpha_{iHc}$  is the value obtained as follows:  $\alpha_{iHc} (\%/\% C.) = \{[(\text{coercivity at } 150^\circ \text{ C.} - \text{coercivity at room temperature } (20^\circ \text{ C.})) / \text{coercivity at room temperature } (20^\circ \text{ C.})] / (150 - 20)\} \times 100$ .

In addition, the rare earth magnet powders obtained by using the present invention's method 1 to 5 and the conventional methods 1 to 5 were compression-molded in a magnetic field to produce anisotropic green compacts. These anisotropic green compacts were set in a hot-pressing apparatus, and hot pressing was carried out under the following conditions: pressing in parallel to the magnetic aligned direction; an Ar gas atmosphere; a temperature of 750°C.; a

pressure of 58.8 MPa; and holding time of 1 minute. The hot pressing was following by quenching so as to produce hot-pressed magnets having a density of 7.5 to 7.7 g/cm<sup>3</sup>. The magnetic properties of the obtained hot-pressed magnets are shown in Table 5. Also, the temperature coefficient of coercivity  $\alpha_{iHc}$  was determined from the result of the magnetic properties measured at 150° C., and those values are shown in Table 5.

Also, to each of the rare earth magnet powders obtained in the present invention's methods 1 to 5 and the conventional methods 1 to 5, an epoxy resin was added at 3 wt % and then mixed therewith, and each of the mixtures was compression-molded while applying a magnetic field of 1.6 MA/m in a compacting direction so as to produce a green compact with a cylindrical shape having a diameter of 10 mm and a height of 7 mm. Subsequently, the obtained cylindrical green compact was hardened in an oven at 150° C. for 2 hours so as to produce a cylindrical bonded magnet having a density of 6.0 to 6.1 g/cm<sup>3</sup>. The obtained bonded magnet was magnetized in pulsed magnetic field of a 70 kOe, and then held for 1,000 hours in an oven maintained at 100° C., and the thermal demagnetizing rates after 3 hours, 100 hours, and 1,000 hours were measured. Those results are shown in Table 5, and the thermal stability was evaluated.

Herein, a “thermal demagnetizing rate” refers to the value obtained as follows: thermal demagnetizing rate (%) = {((total magnetic flux after exposure for a predetermined hours - total magnetic flux before exposure)/total magnetic flux before exposure} × 100. Also, a “thermal demagnetizing rate” can be referred to as an “irreversible flux loss”.

TABLE 2

TABLE 3

| Type                | Remarks | Average particle diameter of rare earth magnet raw material hydride powder obtained by heat-treating ingot in Table 1 in depressurized | Hydrogen-containing raw material mixed powder |            |                     | Amount of Dy/Tb hydride added to rare earth magnet raw material hydride powder (mol %) | Diffusion heat-treatment |                      | Hydrogen desorption |                         |                      |                    |
|---------------------|---------|----------------------------------------------------------------------------------------------------------------------------------------|-----------------------------------------------|------------|---------------------|----------------------------------------------------------------------------------------|--------------------------|----------------------|---------------------|-------------------------|----------------------|--------------------|
|                     |         |                                                                                                                                        | Dy hydride                                    | Tb hydride | Dy—Tb alloy hydride |                                                                                        | Pressure (kPa)           | Holding temp. (° C.) | Holding time (min)  | Ultimate pressure (kPa) | Holding temp. (° C.) | Holding time (min) |
|                     |         | hydrogen, then milling (μm)                                                                                                            |                                               |            |                     |                                                                                        |                          |                      |                     |                         |                      |                    |
| Invention's method  | 1       | Continued from Table 2                                                                                                                 | —                                             | —          | —                   | —                                                                                      | —                        | —                    | —                   | 0.013                   | 820                  | 10                 |
| Conventional method |         |                                                                                                                                        | 300                                           | 0.9        | —                   | —                                                                                      | $1 \times 10^{-4}$       | 820                  | 30                  | $1 \times 10^{-4}$      |                      | 30                 |
| Invention's method  | 2       |                                                                                                                                        | —                                             | —          | —                   | —                                                                                      | —                        | —                    | —                   | 0.013                   | 820                  | 9                  |
| Conventional method |         |                                                                                                                                        | 300                                           | —          | 0.9                 | —                                                                                      | $1 \times 10^{-4}$       | 820                  | 30                  | $1 \times 10^{-4}$      |                      | 30                 |
| Invention's method  | 3       |                                                                                                                                        | —                                             | —          | —                   | —                                                                                      | —                        | —                    | —                   | 0.013                   | 820                  | 10                 |
| Conventional method |         |                                                                                                                                        | 300                                           | —          | —                   | 0.9                                                                                    | $1 \times 10^{-4}$       | 820                  | 30                  | $1 \times 10^{-4}$      |                      | 30                 |
| Invention's method  | 4       |                                                                                                                                        | —                                             | —          | —                   | —                                                                                      | —                        | —                    | —                   | 0.013                   | 820                  | 8                  |
| Conventional method |         |                                                                                                                                        | 300                                           | 0.45       | 0.45                | —                                                                                      | $1 \times 10^{-4}$       | 820                  | 30                  | $1 \times 10^{-4}$      |                      | 30                 |
| Invention's method  | 5       |                                                                                                                                        | —                                             | —          | —                   | —                                                                                      | —                        | —                    | —                   | 0.013                   | 820                  | 11                 |
| Conventional method |         |                                                                                                                                        | 300                                           | 0.3        | 0.3                 | 0.3                                                                                    | $1 \times 10^{-4}$       | 820                  | 30                  | $1 \times 10^{-4}$      |                      | 30                 |

TABLE 4

| Type                | Remarks | Rare earth magnet powder         |                                 |                 |                          |              |     |
|---------------------|---------|----------------------------------|---------------------------------|-----------------|--------------------------|--------------|-----|
|                     |         | EPMA detected intensity          |                                 |                 | Thickness                |              |     |
|                     |         | Peak value near surface (counts) | Peak value near center (counts) | Intensity ratio | of Dy—Tb rich layer (μm) | Coverage (%) |     |
| Invention's method  | 1       | Continued from Table 3           | 1410                            | 811             | 1.74                     | 4.1          | 95  |
| Conventional method |         |                                  | 1180                            | 1176            | 1.00                     | —            | 0   |
| Invention's method  | 2       |                                  | 3929                            | 1854            | 2.12                     | 7.8          | 90  |
| Conventional method |         |                                  | 2160                            | 2182            | 0.99                     | —            | 0   |
| Invention's method  | 3       |                                  | 2677                            | 1394            | 1.92                     | 6.1          | 90  |
| Conventional method |         |                                  | 1685                            | 1668            | 1.01                     | —            | 0   |
| Invention's method  | 4       |                                  | 1650                            | 887             | 1.86                     | 5.9          | 100 |
| Conventional method |         |                                  | 1257                            | 1252            | 1.00                     | —            | 0   |
| Invention's method  | 5       |                                  | 1562                            | 924             | 1.69                     | 5.4          | 95  |
| Conventional method |         |                                  | 1315                            | 1289            | 1.02                     | —            | 0   |

TABLE 5

| Type                | Bonded magnet |            |                            |                         | Hot-pressed magnet |            |                            |                         | Thermal demagnetizing rate for bonded magnet after being held for time indicated below in 100° C. oven (%) |      |       |       |
|---------------------|---------------|------------|----------------------------|-------------------------|--------------------|------------|----------------------------|-------------------------|------------------------------------------------------------------------------------------------------------|------|-------|-------|
|                     | Br (T)        | iHc (MA/m) | BHmax (KJ/m <sup>3</sup> ) | $\alpha_{iHc}$ (%/° C.) | Br (T)             | iHc (MA/m) | BHmax (KJ/m <sup>3</sup> ) | $\alpha_{iHc}$ (%/° C.) |                                                                                                            |      |       |       |
| Invention's method  | 1             | 0.99       | 1.16                       | 188                     | -0.37              | 1.26       | 1.14                       | 283                     | -0.40                                                                                                      | -7.3 | -8.3  | -9.9  |
| Conventional method |               | 0.98       | 1.05                       | 179                     | -0.45              | 1.24       | 1.04                       | 274                     | -0.48                                                                                                      | -8.9 | -11.9 | -17.6 |
| Invention's method  | 2             | 0.94       | 1.67                       | 158                     | -0.35              | 1.18       | 1.66                       | 250                     | -0.37                                                                                                      | -5.1 | -5.8  | -6.8  |
| Conventional method |               | 0.92       | 1.53                       | 150                     | -0.43              | 1.17       | 1.51                       | 242                     | -0.46                                                                                                      | -6.1 | -8.2  | -12.1 |
| Invention's method  | 3             | 0.95       | 1.69                       | 171                     | -0.38              | 1.21       | 1.67                       | 260                     | -0.41                                                                                                      | -5.0 | -5.7  | -6.8  |
| Conventional method |               | 0.94       | 1.52                       | 163                     | -0.44              | 1.19       | 1.55                       | 252                     | -0.47                                                                                                      | -6.0 | -8.0  | -11.8 |
| Invention's method  | 4             | 0.98       | 1.32                       | 185                     | -0.37              | 1.24       | 1.31                       | 271                     | -0.40                                                                                                      | -6.4 | -7.3  | -8.7  |
| Conventional method |               | 0.96       | 1.19                       | 176                     | -0.45              | 1.22       | 1.18                       | 263                     | -0.48                                                                                                      | -7.8 | -10.5 | -15.5 |
| Invention's method  | 5             | 0.94       | 1.28                       | 172                     | -0.38              | 1.20       | 1.27                       | 255                     | -0.41                                                                                                      | -6.6 | -7.5  | -8.9  |
| Conventional method |               | 0.93       | 1.15                       | 164                     | -0.46              | 1.18       | 1.14                       | 247                     | -0.49                                                                                                      | -8.1 | -10.8 | -16.0 |

On the basis of the results shown in Tables 1 to 5, the magnetic properties of the bonded magnets and the hot-pressed magnets produced by using the rare earth magnet powders produced by the present invention's methods 1 to 5, in which a mixed powder was produced by milling a block in an Ar gas atmosphere followed by adding a hydride powder thereto, showed improvements in both coercivity and remanence when compared with the magnetic properties of bonded magnets and hot-pressed magnets produced by using the rare earth magnet powders produced by the conventional methods 1 to 5 in which milling was not carried out and a hydride was not added. Moreover, the temperature coefficient of the coercivity and the thermal demagnetizing rate were both small, indicating that each of the magnets obtained by the present invention's methods also had an excellent thermal stability.

The methods, which determine the depth of the Dy—Tb rich layer from the surface and the surface coverage of the layer by measuring the detected intensities and the ratio thereof in the present invention, are described in detail below using the rare earth magnet powder obtained by the present invention's method 1.

First, the rare earth magnet powder obtained by the present invention's method 1 was embedded in phenolic resin and polished to a mirror surface; then, the elemental distribution of Dy in an internal cross-section of the powder was examined with the EPMA. FIG. 1 shows an image of the elemental distribution of Dy taken at that time. Places having a greater number of bright points indicate a higher Dy content. The presence of numerous bright points near the peripheral edge of the cross-section indicates that the Dy content in a powder particle is higher near the surface than near the center. Therefore, a line analysis of the Dy on a straight line from point A to point B in FIG. 1 was carried out with the EPMA. Mea-

surement at this time was carried out under the following conditions: an acceleration voltage of 15 kV; the minimum electron beam diameter; a dwell time of 1.0 sec/point; and measurement intervals of 1.0  $\mu$ m, and using the Dy L $\alpha$  emission (a wavelength of 0.1909 nm) that is a characteristic X-ray of Dy. The results are shown in FIG. 2. The horizontal axis of the graph represents the migration distance (mm) within the sample, and the vertical axis represents the detected intensity of the Dy L $\alpha$  emission as an X-ray count. A Dy L $\alpha$  emission of 800 counts or more is detected in the portion of the plot extending from the vicinity of 0.01 mm to the vicinity of 0.135 mm that corresponds to a powder particle. In particular, it is apparent that the peak near 0.01 mm (hereinafter referred to as "Peak A") having an intensity of 1440 counts and the peak near 0.135 mm (hereinafter referred to as "Peak B") having an intensity of 1380 counts are strong peaks at both ends, indicating that the Dy content in the powder particle is higher near the surface than near the center. The intensity near the center, which is calculated as the average intensity between 0.051 mm and 0.093 mm (a region which corresponds to  $\frac{1}{3}$  of the powder particle diameter), was 811 counts. Therefore, the intensity ratios of Peak A and Peak B relative to the near-center region were found to be respectively 1.78 and 1.70, and both values were substantially larger than 1.2. When similar line analyses were carried out ten times, each time at a different sample orientation, the detected intensities at 19 places near the surface were found to be at least 1.2 times the detected intensity near the center; therefore, the surface coverage by high Dy content regions was determined to be 95%.

Next, line analysis centered on Peak A was carried out with a dwell time of 1.0 sec and at an as small measurement interval of 20 nm as possible. The results are shown in FIG. 3. The Peak A region was defined as the region where the inten-

sity was at least 1.2 times (973 counts) the detected intensity near the center, the 1.2 times being thought to be of sufficient significance. Then, the Peak A region had a width of 4.1  $\mu\text{m}$ . Analysis by the EPMA was similarly carried out on the magnet powder obtained by the conventional method 1. FIG. 4 shows the results of line analysis at 1.0  $\mu\text{m}$  intervals. The average detected intensity of Dy L $\alpha$  emission near the center was 1176 counts, and the intensity near the surface was 1360 counts in the vicinity of 0.02 mm (hereinafter referred to as "Peak C"), which was less than 1411 counts of 1.2 times the intensity near the center. FIG. 5 shows the results of line analysis at 20 nm intervals. When measured at 20 nm intervals, the intensity of Peak C was in fact 1180 counts which did not differ from the intensity near the center. Thus, it was found that the Dy content near the surface and the Dy content near the center did not have substantial difference.

Likewise, the detected intensities of Dy and Tb near the center and near the surface, the intensity ratio therebetween, the thickness of the Dy—Tb rich layer, and the surface coverage by the Dy—Tb rich layer were determined by analysis with the EPMA for rare earth magnet powders produced by the present invention's methods 2 to 5 and the conventional methods 2 to 5. These values were likewise determined also for rare earth magnet powders produced by the present invention's methods 6 to 30 and the conventional methods 6 to 30 in Examples 2 to 6 described below.

#### Example 2

The present invention's methods 6 to 10 were carried out as follows. Blocks obtained from ingots f to j in Table 1 were milled in an Ar gas atmosphere to the average particle diameters shown in Table 6 so as to produce rare earth magnet alloy raw material powders. To these rare earth magnet alloy raw material powders, a Dy hydride powder, a Tb hydride powder, or a Dy—Tb binary alloy hydride powder, each of which has an average particle diameter of 5  $\mu\text{m}$  was added at the amount shown in Table 6, and then mixed therewith so as to produce mixed powders. The respective mixed powders were then subjected to, in order, hydrogen absorption under the conditions shown in Table 6; hydrogen absorption-decomposition under the conditions shown in Table 6; if necessary, intermediate heat treatment under the conditions shown in Table 7; if necessary, heat treatment in depressurized hydrogen under the conditions shown in Table 7; hydrogen desorption under the conditions shown in Table 8; forcibly cooling to room temperature with Ar gas; and then pulverizing to 300  $\mu\text{m}$  or below, thereby producing rare earth magnet powders.

#### Conventional Example 2

Conventional methods 6 to 10 were carried out as follows. Blocks obtained from ingots f to j in Table 1 were subjected to hydrogen absorption under the same conditions as in Example 2 and shown in Table 6 without milling the blocks nor adding a hydride powder so as to produce a mixed powder, and then were subjected to, in order, hydrogen absorption-decomposition under the same conditions as in Example 2 and shown in Table 6; if necessary, heat treatment in depressurized hydrogen under the conditions shown in Table 7; forcibly cooling to room temperature in Ar gas; and then milling treatment to the average particle diameter shown in Table 8 so as to produce rare earth magnet raw material hydride powders. Then, to these rare earth magnet raw material hydride powders, a Dy hydride powder, a Tb hydride

powder, or a Dy—Tb binary alloy hydride powder, each of which has an average particle diameter of 5  $\mu\text{m}$ , was added at the amount shown in Table 8 and then mixed therewith so as to produce hydrogen-containing raw material mixed powders. Each of these hydrogen-containing raw material mixed powders was subjected to diffusion heat-treating including heating in a vacuum followed by holding under the conditions shown in Table 8; hydrogen desorption under the conditions shown in Table 8; forcibly cooling to room temperature with Ar gas; and then pulverizing to 300  $\mu\text{m}$  or below, thereby producing rare earth magnet powders.

Each of the rare earth magnet powders obtained by using the present invention's methods 6 to 10 and the conventional methods 6 to 10 was embedded in a phenolic resin and polished to a mirror surface, and the detected intensities of near-center and near-surface Dy and/or Tb and the intensity ratio thereof were measured by analysis with the EPMA, thereby determining the values of the depth of the Dy—Tb rich layer from the surface and of the surface coverage by the Dy—Tb rich layer. Those results are given in Table 9.

In addition, to each of the rare earth magnet powders obtained in the present invention's methods 6 to 10 and the conventional methods 6 to 10, an epoxy resin was added at 3 wt % and then mixed therewith, and each of the mixtures was compression-molded in a magnetic field of 1.6 MA/m so as to produce a green compact. The green compact was hardened in an oven at 150° C. for 2 hours so as to produce a bonded magnet having a density of 6.0 to 6.1 g/cm<sup>3</sup>. The magnetic properties of the obtained bonded magnet are shown in Table 10. Also, the temperature coefficient of coercivity  $\alpha_{iHc}$  for each magnet was determined from the result of the magnetic properties measured at 150° C., and those values are shown in Table 10.

Also, to each of the rare earth magnet powders obtained in the present invention's methods 6 to 10 and the conventional methods 6 to 10, an epoxy resin was added at 3 wt % and then mixed therewith, and each of the mixtures was compression-molded while applying a magnetic field of 1.6 MA/m in a compacting direction so as to produce a green compact with a cylindrical shape having a diameter of 10 mm and a height of 7 mm. Subsequently, the obtained cylindrical green compact was hardened in an oven at 150° C. for 2 hours so as to produce a cylindrical bonded magnet having a density of 6.0 to 6.1 g/cm<sup>3</sup>. The obtained the bonded magnet was magnetized in pulsed magnetic field of a 70 kOe, and then held for 1,000 hours in an oven maintained at 100° C., and the thermal demagnetizing rates after 3 hours, 100 hours, and 1,000 hours were measured. Those results are shown in Table 10, and the thermal stability was evaluated.

In addition, the rare earth magnet powders obtained by using the present invention's method 6 to 10 and the conventional methods 6 to 10 were compression-molded in a magnetic field to produce anisotropic green compacts. These anisotropic green compacts were set in a hot-pressing apparatus, and hot pressing was carried out under the following conditions: pressing in parallel to the magnetic aligned direction; an Ar gas atmosphere; a temperature of 750° C.; a pressure of 58.8 MPa; and holding time of 1 minute. The hot pressing was following by quenching so as to produce hot-pressed magnets having a density of 7.5 to 7.7 g/cm<sup>3</sup>. The magnetic properties of the obtained hot-pressed magnets are shown in Table 10. Also, the temperature coefficient of coercivity  $\alpha_{iHc}$  was determined from the result of the magnetic properties measured at 150° C., and those values are shown in Table 10.

TABLE 6

| Type                   | Ingot in<br>Table 1 | Table 1 in Ar<br>atmosphere<br>( $\mu$ m) | Average<br>particle<br>diameter of<br>rare earth<br>magnet raw<br>material<br>powder<br>obtained by<br>milling<br>ingot in | Mixed powder<br>Amount of hydride added<br>to rare earth magnet raw<br>material powder (mol %) | Hydrogen absorption |               |                           | Hydrogen<br>absorption-decomposition |                                      |                          |
|------------------------|---------------------|-------------------------------------------|----------------------------------------------------------------------------------------------------------------------------|------------------------------------------------------------------------------------------------|---------------------|---------------|---------------------------|--------------------------------------|--------------------------------------|--------------------------|
|                        |                     |                                           |                                                                                                                            |                                                                                                | Dry<br>hydride      | Tb<br>hydride | Dy—Tb<br>alloy<br>hydride | Hydrogen<br>Pressure<br>(kPa)        | Holding<br>temp.<br>( $^{\circ}$ C.) | Holding<br>time<br>(min) |
|                        |                     |                                           |                                                                                                                            |                                                                                                |                     |               |                           |                                      |                                      |                          |
| Invention's<br>method  | 6                   | f                                         | 300                                                                                                                        | 0.1                                                                                            | —                   | —             | —                         | 500                                  | 150                                  | 20                       |
| Conventional<br>method |                     |                                           | —                                                                                                                          |                                                                                                | —                   | —             | —                         |                                      |                                      |                          |
| Invention's<br>method  | 7                   | g                                         | 300                                                                                                                        | —                                                                                              | —                   | 1.0           | —                         | 300                                  | 180                                  | 40                       |
| Conventional<br>method |                     |                                           | —                                                                                                                          |                                                                                                | —                   | —             | —                         |                                      |                                      |                          |
| Invention's<br>method  | 8                   | h                                         | 300                                                                                                                        | —                                                                                              | —                   | —             | 2.0                       | 700                                  | 200                                  | 60                       |
| Conventional<br>method |                     |                                           | —                                                                                                                          |                                                                                                | —                   | —             | —                         |                                      |                                      |                          |
| Invention's<br>method  | 9                   | i                                         | 300                                                                                                                        | —                                                                                              | 3.0                 | —             | —                         | 100                                  | 250                                  | 90                       |
| Conventional<br>method |                     |                                           | —                                                                                                                          |                                                                                                | —                   | —             | —                         |                                      |                                      |                          |
| Invention's<br>method  | 10                  | j                                         | 300                                                                                                                        | —                                                                                              | —                   | 5.0           | —                         | 900                                  | 300                                  | 120                      |
| Conventional<br>method |                     |                                           | —                                                                                                                          |                                                                                                | —                   | —             | —                         |                                      |                                      |                          |

TABLE 7

| Type                   | Remarks | Intermediate<br>heat treatment |                                      |                          | Heat treatment in<br>depressurized hydrogen |                                      |                          |
|------------------------|---------|--------------------------------|--------------------------------------|--------------------------|---------------------------------------------|--------------------------------------|--------------------------|
|                        |         | Ar<br>pressure<br>(kPa)        | Holding<br>temp.<br>( $^{\circ}$ C.) | Holding<br>time<br>(min) | Hydrogen<br>pressure<br>(kPa)               | Holding<br>temp.<br>( $^{\circ}$ C.) | Holding<br>time<br>(min) |
|                        |         |                                |                                      |                          |                                             |                                      |                          |
| Invention's<br>method  | 6       | Continued<br>from Table 6      | 500                                  | 820                      | 5                                           | 2.6                                  | 820                      |
| Conventional<br>method |         |                                | —                                    | —                        | —                                           | —                                    | —                        |
| Invention's<br>method  | 7       |                                | —                                    | —                        | 3.9                                         | 820                                  | 120                      |
| Conventional<br>method |         |                                | —                                    | —                        | —                                           | —                                    | —                        |
| Invention's<br>method  | 8       |                                | 700                                  | 840                      | 10                                          | —                                    | —                        |
| Conventional<br>method |         |                                | —                                    | —                        | 3.9                                         | 840                                  | 120                      |
| Invention's<br>method  | 9       |                                | —                                    | —                        | —                                           | —                                    | —                        |
| Conventional<br>method |         |                                | —                                    | —                        | 3.9                                         | 860                                  | 120                      |
| Invention's<br>method  | 10      |                                | 900                                  | 880                      | 8                                           | 8                                    | 880                      |
| Conventional<br>method |         |                                | —                                    | —                        | —                                           | —                                    | 240                      |

TABLE 8

| Type                | Remarks | Average particle diameter of rare earth magnet raw material hydride powder obtained by heat-treating ingot in Table 1 in depressurized | Hydrogen-containing raw material mixed powder |            |                     | Amount of Dy/Tb hydride added to rare earth magnet raw material hydride powder (mol %) | Diffusion heat-treatment |                      | Hydrogen desorption |                         |                      |                    |
|---------------------|---------|----------------------------------------------------------------------------------------------------------------------------------------|-----------------------------------------------|------------|---------------------|----------------------------------------------------------------------------------------|--------------------------|----------------------|---------------------|-------------------------|----------------------|--------------------|
|                     |         |                                                                                                                                        | Dy hydride                                    | Tb hydride | Dy—Tb alloy hydride |                                                                                        | Pressure (kPa)           | Holding temp. (° C.) | Holding time (min)  | Ultimate pressure (kPa) | Holding temp. (° C.) | Holding time (min) |
|                     |         | hydrogen, then milling (μm)                                                                                                            |                                               |            |                     |                                                                                        |                          |                      |                     |                         |                      |                    |
| Invention's method  | 6       | Continued from Table 7                                                                                                                 | —                                             | —          | —                   | —                                                                                      | —                        | —                    | —                   | 0.066                   | 820                  | 12                 |
| Conventional method |         |                                                                                                                                        | 300                                           | 1.0        | —                   | —                                                                                      | $1 \times 10^{-4}$       | 820                  | 30                  | $1 \times 10^{-4}$      |                      | 30                 |
| Invention's method  | 7       |                                                                                                                                        | —                                             | —          | —                   | —                                                                                      | —                        | —                    | —                   | 0.026                   | 820                  | 16                 |
| Conventional method |         |                                                                                                                                        | 300                                           | —          | 1                   | —                                                                                      | $1 \times 10^{-4}$       | 820                  | 30                  | $1 \times 10^{-4}$      |                      | 30                 |
| Invention's method  | 8       |                                                                                                                                        | —                                             | —          | —                   | —                                                                                      | —                        | —                    | —                   | 0.013                   | 820                  | 9                  |
| Conventional method |         |                                                                                                                                        | 300                                           | —          | —                   | 2                                                                                      | $1 \times 10^{-4}$       | 840                  | 30                  | $1 \times 10^{-4}$      |                      | 30                 |
| Invention's method  | 9       |                                                                                                                                        | —                                             | —          | —                   | —                                                                                      | —                        | —                    | —                   | 0.013                   | 820                  | 7                  |
| Conventional method |         |                                                                                                                                        | 300                                           | 3          | —                   | —                                                                                      | $1 \times 10^{-4}$       | 860                  | 30                  | $1 \times 10^{-4}$      |                      | 30                 |
| Invention's method  | 10      |                                                                                                                                        | —                                             | —          | —                   | —                                                                                      | —                        | —                    | —                   | 0.013                   | 820                  | 10                 |
| Conventional method |         |                                                                                                                                        | 300                                           | —          | 5                   | —                                                                                      | $1 \times 10^{-4}$       | 880                  | 30                  | $1 \times 10^{-4}$      |                      | 30                 |

TABLE 9

| Type                | Remarks | Rare earth magnet powder         |                                 |                 |                          |              |     |
|---------------------|---------|----------------------------------|---------------------------------|-----------------|--------------------------|--------------|-----|
|                     |         | EPMA detected intensity          |                                 |                 | Thickness                |              |     |
|                     |         | Peak value near surface (counts) | Peak value near center (counts) | Intensity ratio | of Dy—Tb rich layer (μm) | Coverage (%) |     |
| Invention's method  | 6       | Continued from Table 8           | 1756                            | 1451            | 1.21                     | 0.1          | 70  |
| Conventional method |         |                                  | 1447                            | 1492            | 0.97                     | —            | 0   |
| Invention's method  | 7       |                                  | 3344                            | 1827            | 1.83                     | 6.8          | 95  |
| Conventional method |         |                                  | 2367                            | 2233            | 1.06                     | —            | 0   |
| Invention's method  | 8       |                                  | 2857                            | 1043            | 2.74                     | 10.1         | 100 |
| Conventional method |         |                                  | 2076                            | 1854            | 1.12                     | —            | 0   |
| Invention's method  | 9       |                                  | 4588                            | 1230            | 3.73                     | 20.7         | 100 |
| Conventional method |         |                                  | 2274                            | 1960            | 1.16                     | —            | 0   |
| Invention's method  | 10      |                                  | 17959                           | 3896            | 4.61                     | 25.6         | 100 |
| Conventional method |         |                                  | 7286                            | 5923            | 1.23                     | 1.0          | 20  |

TABLE 10

| Type                | Bonded magnet |            |                            |                         | Hot-pressed magnet |            |                            |                         | Thermal demagnetizing rate for bonded magnet after being held for time indicated below in 100° C. oven (%) |      |       |       |
|---------------------|---------------|------------|----------------------------|-------------------------|--------------------|------------|----------------------------|-------------------------|------------------------------------------------------------------------------------------------------------|------|-------|-------|
|                     | Br (T)        | iHc (MA/m) | BHmax (KJ/m <sup>3</sup> ) | $\alpha_{iHc}$ (%/° C.) | Br (T)             | iHc (MA/m) | BHmax (KJ/m <sup>3</sup> ) | $\alpha_{iHc}$ (%/° C.) |                                                                                                            |      |       |       |
| Invention's method  | 6             | 0.93       | 1.74                       | 158                     | -0.40              | 1.17       | 1.73                       | 245                     | -0.43                                                                                                      | -4.9 | -5.5  | -6.5  |
| Conventional method |               | 0.91       | 1.73                       | 149                     | -0.41              | 1.15       | 1.71                       | 236                     | -0.44                                                                                                      | -5.4 | -7.2  | -10.7 |
| Invention's method  | 7             | 0.95       | 1.78                       | 166                     | -0.38              | 1.20       | 1.76                       | 255                     | -0.41                                                                                                      | -4.8 | -5.4  | -6.4  |
| Conventional method |               | 0.93       | 1.66                       | 158                     | -0.43              | 1.18       | 1.65                       | 247                     | -0.46                                                                                                      | -5.6 | -7.5  | -11.1 |
| Invention's method  | 8             | 0.95       | 1.48                       | 172                     | -0.36              | 1.21       | 1.46                       | 259                     | -0.39                                                                                                      | -5.7 | -6.5  | -7.7  |
| Conventional method |               | 0.94       | 1.25                       | 165                     | -0.42              | 1.19       | 1.24                       | 252                     | -0.45                                                                                                      | -7.5 | -10.0 | -14.8 |
| Invention's method  | 9             | 0.94       | 1.53                       | 165                     | -0.35              | 1.19       | 1.51                       | 252                     | -0.37                                                                                                      | -5.5 | -6.3  | -7.5  |
| Conventional method |               | 0.93       | 1.30                       | 160                     | -0.41              | 1.18       | 1.38                       | 247                     | -0.44                                                                                                      | -6.7 | -9.0  | -13.3 |
| Invention's method  | 10            | 0.96       | 2.53                       | 166                     | -0.34              | 1.22       | 2.51                       | 265                     | -0.36                                                                                                      | -3.3 | -3.8  | -4.5  |
| Conventional method |               | 0.96       | 2.04                       | 164                     | -0.40              | 1.22       | 2.02                       | 263                     | -0.43                                                                                                      | -4.6 | -6.1  | -9.1  |

On the basis of the results shown in Table 1 and Table 6 to 10, the magnetic properties of the bonded magnets and the hot-pressed magnets produced by using the rare earth magnet powders produced by the present invention's methods 6 to 10, in which a mixed powder was produced by milling a block in an Ar gas atmosphere followed by adding a hydride powder thereto, showed improvements in both coercivity and remanence when compared with the magnetic properties of bonded magnets and hot-pressed magnets produced by using the rare earth magnet powders produced by the conventional methods 6 to 10 in which milling was not carried out and a hydride was not added. Moreover, the temperature coefficient of the coercivity and the thermal demagnetizing rate were both small, indicating that each of the magnets obtained by the present invention's methods also had an excellent thermal stability.

### Example 3

The present invention's methods 11 to 15 were carried out as follows. Blocks obtained from ingots k to o in Table 1 were milled in an Ar gas atmosphere to the average particle diameters shown in Table 11 so as to produce rare earth magnet alloy raw material powders. To these rare earth magnet alloy raw material powders, a Dy hydride powder, a Tb hydride powder, or a Dy—Tb binary alloy hydride powder, each of which has an average particle diameter of 5  $\mu\text{m}$  was added at the amount shown in Table 11, and then mixed therewith so as to produce mixed powders. The respective mixed powders were then subjected to, in order, hydrogen absorption under the conditions shown in Table 11; hydrogen absorption-decomposition under the conditions shown in Table 11; if necessary, intermediate heat treatment under the conditions shown in Table 11; if necessary, heat treatment in depressurized hydrogen under the conditions shown in Table 11; hydrogen desorption under the conditions shown in Table 12; forc-

ibly cooling to room temperature with Ar gas; and then pulverizing to 300  $\mu\text{m}$  or below, thereby producing rare earth magnet powders.

### Conventional Example 3

Conventional methods 11 to 15 were carried out as follows. Blocks obtained from ingots k to o in Table 1 were subjected to hydrogen absorption under the same conditions as in Example 3 and shown in Table 11 without milling the blocks nor adding a hydride powder so as to produce a mixed powder, and then were subjected to, in order, hydrogen absorption-decomposition under the same conditions as in Example 3 and shown in Table 11; if necessary, heat treatment in depressurized hydrogen under the conditions shown in Table 11; forcibly cooling to room temperature in Ar gas; and then milling treatment to the average particle diameter shown in Table 12 so as to produce rare earth magnet raw material hydride powders. Then, to these rare earth magnet raw material hydride powders, a Dy hydride powder, a Tb hydride powder, or a Dy—Tb binary alloy hydride powder, each of which has an average particle diameter of 5  $\mu\text{m}$ , was added at the amount shown in Table 12 and then mixed therewith so as to produce hydrogen-containing raw material mixed powders. Each of these hydrogen-containing raw material mixed powders was subjected to diffusion heat-treating including heating in a vacuum followed by holding under the conditions shown in Table 12; hydrogen desorption under the conditions shown in Table 12; forcibly cooling to room temperature with Ar gas; and then pulverizing to 300  $\mu\text{m}$  or below, thereby producing rare earth magnet powders.

Each of the rare earth magnet powders obtained by using the present invention's methods 11 to 15 and the conventional methods 11 to 15 was embedded in a phenolic resin and polished to a mirror surface, and the detected intensities of near-center and near-surface Dy and/or Tb and the intensity ratio thereof were measured by analysis with the EPMA,

thereby determining the values of the depth of the Dy—Tb rich layer from the surface and of the surface coverage by the Dy—Tb rich layer. Those results are given in Table 13.

To each of the rare earth magnet powders obtained in the present invention's methods 11 to 15 and the conventional methods 11 to 15, an epoxy resin was added at 3 wt % and then mixed therewith, and each of the mixtures was compression-molded in a magnetic field of 1.6 MA/m so as to produce a green compact. The green compact was hardened in an oven at 150° C. for 2 hours so as to produce a bonded magnet having a density of 6.0 to 6.1 g/cm<sup>3</sup>. The magnetic properties of the obtained bonded magnet are shown in Table 14. Also, the temperature coefficient of coercivity  $\alpha_{iHc}$  for each magnet was determined from the result of the magnetic properties measured at 150° C., and those values are shown in Table 14.

Also, to each of the rare earth magnet powders obtained in the present invention's methods 11 to 15 and the conventional methods 11 to 15, an epoxy resin was added at 3 wt % and then mixed therewith, and each of the mixtures was compression-molded while applying a magnetic field of 1.6 MA/m in a compacting direction so as to produce a green compact with a cylindrical shape having a diameter of 10 mm and a height of 7 mm. Subsequently, the obtained cylindrical green compact was hardened in an oven at 150° C. for 2 hours so as to

produce a cylindrical bonded magnet having a density of 6.0 to 6.1 g/cm<sup>3</sup>. The obtained the bonded magnet was magnetized in pulsed magnetic field of a 70 kOe, and then held for 1,000 hours in an oven maintained at 100° C., and the thermal demagnetizing rates after 3 hours, 100 hours, and 1,000 hours were measured. Those results are shown in Table 14, and the thermal stability was evaluated.

In addition, the rare earth magnet powders obtained by using the present invention's method 11 to 15 and the conventional methods 11 to 15 were compression-molded in a magnetic field to produce anisotropic green compacts. These anisotropic green compacts were set in a hot-pressing apparatus, and hot pressing was carried out under the following conditions: pressing in parallel to the magnetic aligned direction; an Ar gas atmosphere; a temperature of 750° C.; a pressure of 58.8 MPa; and holding time of 1 minute. The hot pressing was followed by quenching so as to produce hot-pressed magnets having a density of 7.5 to 7.7 g/cm<sup>3</sup>. The magnetic properties of the obtained hot-pressed magnets are shown in Table 14. Also, the temperature coefficient of coercivity  $\alpha_{,Hc}$  was determined from the result of the magnetic properties measured at 150° C., and those values are shown in Table 14.

TABLE 11

TABLE 12

| Type                | Remarks | Average particle diameter of rare earth magnet raw material hydride powder obtained by heat-treating ingot in Table 1 in depressurized hydrogen, then milling (μm) | Hydrogen-containing raw material mixed powder |            |                     | Diffusion heat-treatment | Hydrogen desorption |                      |                    |                         |                      |                    |
|---------------------|---------|--------------------------------------------------------------------------------------------------------------------------------------------------------------------|-----------------------------------------------|------------|---------------------|--------------------------|---------------------|----------------------|--------------------|-------------------------|----------------------|--------------------|
|                     |         |                                                                                                                                                                    | Dy hydride                                    | Tb hydride | Dy—Tb alloy hydride |                          | Pressure (kPa)      | Holding temp. (° C.) | Holding time (min) | Ultimate pressure (kPa) | Holding temp. (° C.) | Holding time (min) |
| Invention's method  | 11      | Continued from Table 11                                                                                                                                            | —                                             | —          | —                   | —                        | —                   | 0.013                | 820                | 8                       |                      |                    |
| Conventional method |         |                                                                                                                                                                    | 10                                            | 0.5        | —                   | —                        | $1 \times 10^{-4}$  | 820                  | 30                 | $1 \times 10^{-4}$      |                      | 30                 |
| Invention's method  | 12      |                                                                                                                                                                    | —                                             | —          | —                   | —                        | —                   | —                    | —                  | 0.013                   |                      | 13                 |
| Conventional method |         |                                                                                                                                                                    | 50                                            | —          | —                   | 1.5                      | $1 \times 10^{-4}$  | 820                  | 30                 | $1 \times 10^{-4}$      |                      | 30                 |
| Invention's method  | 13      |                                                                                                                                                                    | —                                             | —          | —                   | —                        | —                   | —                    | —                  | 0.013                   |                      | 7                  |
| Conventional method |         |                                                                                                                                                                    | 100                                           | 1          | 1                   | —                        | $1 \times 10^{-4}$  | 820                  | 30                 | $1 \times 10^{-4}$      |                      | 30                 |
| Invention's method  | 14      |                                                                                                                                                                    | —                                             | —          | —                   | —                        | —                   | —                    | —                  | 0.013                   |                      | 9                  |
| Conventional method |         |                                                                                                                                                                    | 200                                           | —          | 2                   | 2                        | $1 \times 10^{-4}$  | 820                  | 30                 | $1 \times 10^{-4}$      |                      | 30                 |
| Invention's method  | 15      |                                                                                                                                                                    | —                                             | —          | —                   | —                        | —                   | —                    | —                  | 0.013                   |                      | 12                 |
| Conventional method |         |                                                                                                                                                                    | 500                                           | 2          | —                   | —                        | $1 \times 10^{-4}$  | 820                  | 30                 | $1 \times 10^{-4}$      |                      | 30                 |

TABLE 13

| Type                | Remarks | Rare earth magnet powder         |                                 |                 |                          |              |     |
|---------------------|---------|----------------------------------|---------------------------------|-----------------|--------------------------|--------------|-----|
|                     |         | EPMA detected intensity          |                                 |                 | Thickness                |              |     |
|                     |         | Peak value near surface (counts) | Peak value near center (counts) | Intensity ratio | of Dy—Tb rich layer (μm) | Coverage (%) |     |
| Invention's method  | 11      | Continued from Table 12          | 2386                            | 1549            | 1.54                     | 4.9          | 85  |
| Conventional method |         |                                  | 1760                            | 1752            | 1.00                     | —            | 0   |
| Invention's method  | 12      |                                  | 3071                            | 1458            | 2.10                     | 7.8          | 100 |
| Conventional method |         |                                  | 2253                            | 2067            | 1.09                     | —            | 0   |
| Invention's method  | 13      |                                  | 2727                            | 1330            | 2.05                     | 11.4         | 100 |
| Conventional method |         |                                  | 2017                            | 1817            | 1.11                     | —            | 0   |
| Invention's method  | 14      |                                  | 8936                            | 2377            | 3.76                     | 20.9         | 100 |
| Conventional method |         |                                  | 4054                            | 3350            | 1.21                     | 0.5          | 10  |
| Invention's method  | 15      |                                  | 3089                            | 953             | 3.24                     | 12.0         | 100 |
| Conventional method |         |                                  | 1627                            | 1440            | 1.13                     | —            | 0   |

TABLE 14

| Type                | Bonded magnet |            |                            |                         | Hot-pressed magnet |            |                            |                         | Thermal demagnetizing rate for bonded magnet after being held for time indicated below in 100° C. oven (%) |           |             |
|---------------------|---------------|------------|----------------------------|-------------------------|--------------------|------------|----------------------------|-------------------------|------------------------------------------------------------------------------------------------------------|-----------|-------------|
|                     | Br (T)        | iHc (MA/m) | BHmax (KJ/m <sup>3</sup> ) | $\alpha_{iHc}$ (%/° C.) | Br (T)             | iHc (MA/m) | BHmax (KJ/m <sup>3</sup> ) | $\alpha_{iHc}$ (%/° C.) | 3 hours                                                                                                    | 100 hours | 1,000 hours |
| Invention's method  | 11            | 0.95       | 1.70                       | 160                     | -0.39              | 1.20       | 1.68                       | 256                     | -0.42                                                                                                      | -5.0      | -5.7 -6.7   |
| Conventional method |               | 0.93       | 1.61                       | 152                     | -0.42              | 1.18       | 1.59                       | 247                     | -0.45                                                                                                      | -5.8      | -7.8 -11.5  |
| Invention's method  | 12            | 0.93       | 1.73                       | 157                     | -0.37              | 1.18       | 1.71                       | 249                     | -0.40                                                                                                      | -4.9      | -5.6 -6.6   |
| Conventional method |               | 0.92       | 1.58                       | 150                     | -0.43              | 1.17       | 1.56                       | 242                     | -0.46                                                                                                      | -5.9      | -7.9 -11.7  |
| Invention's method  | 13            | 0.96       | 1.47                       | 171                     | -0.36              | 1.22       | 1.45                       | 264                     | -0.39                                                                                                      | -5.8      | -6.6 -7.8   |
| Conventional method |               | 0.95       | 1.31                       | 165                     | -0.44              | 1.20       | 1.30                       | 258                     | -0.47                                                                                                      | -7.1      | -9.5 -14.1  |
| Invention's method  | 14            | 0.95       | 2.13                       | 165                     | -0.36              | 1.20       | 2.11                       | 256                     | -0.39                                                                                                      | -4.0      | -4.5 -5.4   |
| Conventional method |               | 0.94       | 1.79                       | 161                     | -0.43              | 1.19       | 1.77                       | 252                     | -0.46                                                                                                      | -5.2      | -7.0 -10.3  |
| Invention's method  | 15            | 0.97       | 1.43                       | 179                     | -0.36              | 1.23       | 1.42                       | 270                     | -0.39                                                                                                      | -5.9      | -6.7 -8.0   |
| Conventional method |               | 0.96       | 1.23                       | 172                     | -0.45              | 1.22       | 1.22                       | 263                     | -0.48                                                                                                      | -7.6      | -10.1 -15.0 |

On the basis of the results shown in Table 1 and Table 11 to 14, the magnetic properties of the bonded magnets and the hot-pressed magnets produced by using the rare earth magnet powders produced by the present invention's methods 11 to 15, in which a mixed powder was produced by milling a block in an Ar gas atmosphere followed by adding a hydride powder thereto, showed improvements in both coercivity and remanence when compared with the magnetic properties of bonded magnets and hot-pressed magnets produced by using the rare earth magnet powders produced by the conventional methods 11 to 15 in which milling was not carried out and a hydride was not added. Moreover, the temperature coefficient of the coercivity and the thermal demagnetizing rate were both small, indicating that each of the magnets obtained by the present invention's methods also had an excellent thermal stability.

#### Example 4

The present invention's methods 16 to 20 were carried out as follows. Blocks obtained from ingots a to e in Table 1 were subjected to hydrogen absorption under the conditions shown in Table 15. Then, these blocks subjected to the hydrogen absorption were milled to the average particle diameters shown in Table 15 so as to produce hydrogen-absorbing rare earth magnet alloy raw material powders. To these hydrogen-absorbing rare earth magnet alloy raw material powders, a Dy hydride powder, a Tb hydride powder, or a Dy-Tb binary alloy hydride powder, each of which has an average particle diameter of 5  $\mu$ m was added at the amount shown in Table 15, and then mixed therewith so as to produce hydrogen-containing raw material mixed powders. The respective hydrogen-containing raw material mixed powders were then subjected to, in order, hydrogen absorption-decomposition under the conditions shown in Table 15; if necessary, intermediate heat treatment under the conditions shown in Table 15; if necessary, heat treatment in depressurized hydrogen under the con-

ditions shown in Table 15; hydrogen desorption under the conditions shown in Table 16; forcibly cooling to room temperature with Ar gas; and then pulverizing to 300  $\mu$ m or below, thereby producing rare earth magnet powders.

#### Conventional Example 4

Conventional methods 16 to 20 were carried out as follows. Blocks obtained from ingots a to e in Table 1 were subjected to hydrogen absorption under the conditions as shown in Table 15 followed by hydrogen absorption-decomposition under the same conditions as in Example 4 and shown in Table 15 without milling the blocks nor adding a hydride powder so as not to produce a hydrogen-containing raw material mixed powder, and then were subjected to, in order, if necessary, heat treatment in depressurized hydrogen under the conditions shown in Table 15; forcibly cooling to room temperature in Ar gas; and then milling treatment to the average particle diameter shown in Table 16 so as to produce rare earth magnet raw material hydride powders. To these rare earth magnet raw material hydride powders, a Dy hydride powder, a Tb hydride powder, or a Dy-Tb binary alloy hydride powder, each of which has an average particle diameter of 5  $\mu$ m, was added at the amount shown in Table 16 and then mixed therewith so as to produce hydrogen-containing raw material mixed powders. Each of these hydrogen-containing raw material mixed powders was subjected to diffusion heat-treating including heating in a vacuum followed by holding under the conditions shown in Table 16; hydrogen desorption under the conditions shown in Table 16; forcibly cooling to room temperature with Ar gas; and then pulverizing to 300  $\mu$ m or below, thereby producing rare earth magnet powders.

Each of the rare earth magnet powders obtained by using the present invention's methods 16 to 20 and the conventional methods 16 to 20 was embedded in a phenolic resin and polished to a mirror surface, and the detected intensities of

near-center and near-surface Dy and/or Tb, and the intensity ratio thereof were measured by analysis with the EPMA, thereby determining the values of the depth of the Dy—Tb rich layer from the surface and of the surface coverage by the Dy—Tb rich layer. Those results are given in Table 17.

As an example, FIG. 6 shows an image of the elemental distribution of Dy taken when the rare earth magnet powder obtained by the present invention's method 16 was embedded in phenolic resin and polished to a mirror surface; then, the elemental distribution of Dy in an internal cross-section of the powder was examined with the EPMA. The presence of numerous bright points near the peripheral edge of the cross-section indicates that the Dy content in a powder particle is higher near the surface than near the center. FIG. 7 shows the results of a line analysis of Dy actually carried out with the EPMA on a straight line from point E to point F in FIG. 6. According to FIG. 7, strong peaks appear at both ends, indicating that the Dy content in the powder particle is higher near the surface than near the center. The average detected intensity of the peaks at both ends was 1412 counts, and the average detected intensity in a region near the center corresponding to  $\frac{1}{3}$  of the powder particle diameter was 915 counts; thus, the ratio of the intensity near the surface relative to the intensity near the center was 1.54. From the result of similar line analyses which were carried out ten times, each time at a different sample orientation, the surface coverage was found to be 95%. Also, from the result of scanning the peaks at both ends at a fine interval, the region where the intensity was at least 1.2 times the detected intensity near the center was found to have a width of 4.5  $\mu\text{m}$ .

The values shown in Table 17 were obtained in this way from the measurement results for the rare earth magnet powder produced by the present invention's method 16 and from measurement results for the rare earth magnet powders produced also by the present invention's method 17 to 20 and the conventional methods 16 to 20.

In addition, to each of the rare earth magnet powders obtained in the present invention's methods 16 to 20 and the conventional methods 16 to 20, an epoxy resin was added at 3 wt % and then mixed therewith, and each of the mixtures was compression-molded in a magnetic field of 1.6 MA/m so as to produce a green compact. The green compact was hardened in an oven at 150° C. for 2 hours so as to produce a bonded magnet having a density of 6.0 to 6.1 g/cm<sup>3</sup>. The magnetic properties of the obtained bonded magnet are shown in Table 18. Also, the temperature coefficient of coerc-

civity  $\alpha_{Hc}$  for each magnet was determined from the result of the magnetic properties measured at 150°C., and those values are shown in Table 18. Herein, the temperature coefficient of coercivity  $\alpha_{Hc}$  is the value obtained as follows:  $\alpha_{Hc}$  (%)<sup>5</sup> C.) = [(coercivity at 150°C. - coercivity at room temperature (20°C.)) / coercivity at room temperature (20°C.)] / (150 - 20) × 100.

In addition, the rare earth magnet powders obtained by using the present invention's method 16 to 20 and the conventional methods 16 to 20 were compression-molded in a magnetic field to produce anisotropic green compacts. These anisotropic green compacts were set in a hot-pressing apparatus, and hot pressing was carried out under the following conditions: pressing in parallel to the magnetic aligned direction; an Ar gas atmosphere; a temperature of 750° C.; a pressure of 58.8 MPa; and holding time of 1 minute. The hot pressing was followed by quenching so as to produce hot-pressed magnets having a density of 7.5 to 7.7 g/cm<sup>3</sup>. The magnetic properties of the obtained hot-pressed magnets are shown in Table 18. Also, the temperature coefficient of coercivity  $\alpha_{IHc}$  was determined from the result of the magnetic properties measured at 150° C., and those values are shown in Table 18.

25 Also, to each of the rare earth magnet powders obtained in the present invention's methods 16 to 20 and the conventional methods 16 to 20, an epoxy resin was added at 3 wt % and then mixed therewith, and each of the mixtures was compression-molded while applying a magnetic field of 1.6 MA/m in a compacting direction so as to produce a green compact with a cylindrical shape having a diameter of 10 mm and a height of 7 mm. Subsequently, the obtained cylindrical green compact was hardened in an oven at 150° C. for 2 hours so as to produce a cylindrical bonded magnet having a density of 6.0  
30 to 6.1 g/cm<sup>3</sup>. To determine their magnetic properties, the obtained the bonded magnet was magnetized in pulsed magnetic field of a 70 kOe, and then held for 1,000 hours in an oven maintained at 100° C., and the thermal demagnetizing rates after 3 hours, 100 hours, and 1,000 hours were measured.  
35 Those results are shown in Table 18, and the thermal stability was evaluated.  
40

Herein, a “thermal demagnetizing rate” refers to the value obtained as follows: thermal demagnetizing rate (%) = { (total magnetic flux after exposure for a predetermined hours - total magnetic flux before exposure) / total magnetic flux before exposure } × 100.

TABLE 15

TABLE 15-continued

| Type                | Ingot | Average particle diameter of rare earth magnet raw material powder obtained by milling ingot in |                        | Mixed powder                                              |            | Hydrogen absorption | Intermediate heat treatment |                        |                      | Heat treatment in depressurized hydrogen |                         |                      |                    |     |
|---------------------|-------|-------------------------------------------------------------------------------------------------|------------------------|-----------------------------------------------------------|------------|---------------------|-----------------------------|------------------------|----------------------|------------------------------------------|-------------------------|----------------------|--------------------|-----|
|                     |       | Table 1 in Ar atmosphere (μm)                                                                   |                        | Amount of hydride added to rare earth magnet raw material |            |                     | Hydrogen                    |                        |                      | Hydrogen                                 |                         |                      |                    |     |
|                     |       | in Table 1 absorption                                                                           | Hydrogen               | Dy hydride                                                | Tb hydride | Dy—Tb alloy         | Hydride decomposition       | Ar pressure (kPa)      | Holding temp. (° C.) | Holding time (min)                       | Hydrogen pressure (kPa) | Holding temp. (° C.) | Holding time (min) |     |
| Invention's method  | 17    | b                                                                                               | Holding temp.: 150° C. | 300                                                       | —          | 0.9                 | —                           | Holding temp.: 820° C. | —                    | —                                        | 3.9                     | 820                  | 120                |     |
| Conventional method |       |                                                                                                 | Holding time: 20 min   | —                                                         | —          | —                   | —                           | 200                    | 820                  | 5                                        | —                       | —                    | —                  |     |
| Invention's method  | 18    | c                                                                                               | —                      | 300                                                       | —          | —                   | 0.9                         | —                      | —                    | —                                        | 3.9                     | 820                  | 120                |     |
| Conventional method |       |                                                                                                 | —                      | —                                                         | —          | —                   | —                           | —                      | —                    | —                                        | 3.9                     | 820                  | 120                |     |
| Invention's method  | 19    | d                                                                                               | —                      | 300                                                       | 0.45       | 0.45                | —                           | —                      | —                    | —                                        | —                       | —                    | —                  |     |
| Conventional method |       |                                                                                                 | —                      | —                                                         | —          | —                   | —                           | —                      | —                    | —                                        | 3.9                     | 820                  | 120                |     |
| Invention's method  | 20    | e                                                                                               | —                      | 300                                                       | 0.3        | 0.3                 | 0.3                         | —                      | 200                  | 820                                      | 5                       | 3.9                  | 820                | 120 |
| Conventional method |       |                                                                                                 | —                      | —                                                         | —          | —                   | —                           | —                      | —                    | —                                        | —                       | —                    | —                  |     |

TABLE 16

| Type                | Remarks | Average particle diameter of rare earth magnet raw material hydride powder obtained by heat-treating ingot in Table 1 in depressurized hydrogen, then milling (μm) |            | Hydrogen-containing raw material mixed powder |                       | Hydrogen absorption | Diffusion heat-treatment |                      |                    | Hydrogen desorption     |                      |                    |
|---------------------|---------|--------------------------------------------------------------------------------------------------------------------------------------------------------------------|------------|-----------------------------------------------|-----------------------|---------------------|--------------------------|----------------------|--------------------|-------------------------|----------------------|--------------------|
|                     |         | Dy hydride                                                                                                                                                         | Tb hydride | Dy—Tb alloy                                   | Hydride decomposition |                     | Pressure (kPa)           | Holding temp. (° C.) | Holding time (min) | Ultimate pressure (kPa) | Holding temp. (° C.) | Holding time (min) |
|                     |         | hydrogen, then milling (μm)                                                                                                                                        | (μm)       | (μm)                                          | (μm)                  |                     | (μm)                     | (μm)                 | (μm)               | (μm)                    | (μm)                 | (μm)               |
| Invention's method  | 16      | Continued from Table 15                                                                                                                                            | —          | —                                             | —                     | —                   | —                        | —                    | —                  | 0.013                   | 820                  | 10                 |
| Conventional method |         |                                                                                                                                                                    | 300        | 0.9                                           | —                     | —                   | 1 × 10 <sup>-4</sup>     | 820                  | 30                 | 1 × 10 <sup>-4</sup>    | 820                  | 30                 |
| Invention's method  | 17      | —                                                                                                                                                                  | —          | —                                             | —                     | —                   | —                        | —                    | —                  | 0.013                   | 820                  | 9                  |
| Conventional method |         |                                                                                                                                                                    | 300        | —                                             | 0.9                   | —                   | 1 × 10 <sup>-4</sup>     | 820                  | 30                 | 1 × 10 <sup>-4</sup>    | 820                  | 30                 |
| Invention's method  | 18      | —                                                                                                                                                                  | —          | —                                             | —                     | —                   | —                        | —                    | —                  | 0.013                   | 820                  | 10                 |
| Conventional method |         |                                                                                                                                                                    | 300        | —                                             | —                     | 0.9                 | 1 × 10 <sup>-4</sup>     | 820                  | 30                 | 1 × 10 <sup>-4</sup>    | 820                  | 30                 |
| Invention's method  | 19      | —                                                                                                                                                                  | —          | —                                             | —                     | —                   | —                        | —                    | —                  | 0.013                   | 820                  | 8                  |
| Conventional method |         |                                                                                                                                                                    | 300        | 0.45                                          | 0.45                  | —                   | 1 × 10 <sup>-4</sup>     | 820                  | 30                 | 1 × 10 <sup>-4</sup>    | 820                  | 30                 |
| Invention's method  | 20      | —                                                                                                                                                                  | —          | —                                             | —                     | —                   | —                        | —                    | —                  | 0.013                   | 820                  | 11                 |
| Conventional method |         |                                                                                                                                                                    | 300        | 0.3                                           | 0.3                   | 0.3                 | 1 × 10 <sup>-4</sup>     | 820                  | 30                 | 1 × 10 <sup>-4</sup>    | 820                  | 30                 |

TABLE 17

|                     |         | Rare earth magnet powder         |                                 |                 |                          |              |     |
|---------------------|---------|----------------------------------|---------------------------------|-----------------|--------------------------|--------------|-----|
| Type                | Remarks | EPMA detected intensity          |                                 |                 | Thickness                |              |     |
|                     |         | Peak value near surface (counts) | Peak value near center (counts) | Intensity ratio | of Dy—Tb rich layer (μm) | Coverage (%) |     |
| Invention's method  | 16      | Continued from Table 16          | 1412                            | 915             | 1.54                     | 4.5          | 95  |
| Conventional method |         |                                  | 1180                            | 1176            | 1.00                     | —            | 0   |
| Invention's method  | 17      |                                  | 3880                            | 1813            | 2.14                     | 7.9          | 95  |
| Conventional method |         |                                  | 2160                            | 2182            | 0.99                     | —            | 0   |
| Invention's method  | 18      |                                  | 2694                            | 1361            | 1.98                     | 6.3          | 90  |
| Conventional method |         |                                  | 1685                            | 1668            | 1.01                     | —            | 0   |
| Invention's method  | 19      |                                  | 1676                            | 842             | 1.99                     | 6.3          | 95  |
| Conventional method |         |                                  | 1257                            | 1252            | 1.00                     | —            | 0   |
| Invention's method  | 20      |                                  | 1494                            | 879             | 1.70                     | 5.4          | 100 |
| Conventional method |         |                                  | 1315                            | 1289            | 1.02                     | —            | 0   |

TABLE 18

| Type                | Bonded magnet |            |                            |                         | Hot-pressed magnet |            |                            |                         | Thermal demagnetizing rate for bonded magnet after being held for time indicated below in 100° C. oven (%) |           |             |       |
|---------------------|---------------|------------|----------------------------|-------------------------|--------------------|------------|----------------------------|-------------------------|------------------------------------------------------------------------------------------------------------|-----------|-------------|-------|
|                     | Br (T)        | iHc (MA/m) | BHmax (KJ/m <sup>3</sup> ) | $\alpha_{iHc}$ (%/° C.) | Br (T)             | iHc (MA/m) | BHmax (KJ/m <sup>3</sup> ) | $\alpha_{iHc}$ (%/° C.) | 3 hours                                                                                                    | 100 hours | 1,000 hours |       |
| Invention's method  | 16            | 1.00       | 1.15                       | -0.37                   | 1.26               | 1.14       | 283                        | -0.40                   | -7.6                                                                                                       | -8.7      | -10.3       |       |
| Conventional method |               | 0.98       | 1.05                       | 179                     | -0.45              | 1.24       | 1.04                       | 274                     | -0.48                                                                                                      | -8.9      | -11.9       | -17.6 |
| Invention's method  | 17            | 0.94       | 1.67                       | 159                     | -0.35              | 1.19       | 1.65                       | 251                     | -0.37                                                                                                      | -5.2      | -6.0        | -7.1  |
| Conventional method |               | 0.92       | 1.53                       | 150                     | -0.43              | 1.17       | 1.51                       | 242                     | -0.46                                                                                                      | -6.1      | -8.2        | -12.1 |
| Invention's method  | 18            | 0.96       | 1.69                       | 173                     | -0.38              | 1.21       | 1.67                       | 262                     | -0.41                                                                                                      | -5.2      | -5.9        | -7.0  |
| Conventional method |               | 0.94       | 1.57                       | 163                     | -0.44              | 1.19       | 1.55                       | 252                     | -0.47                                                                                                      | -6.0      | -8.0        | -11.8 |
| Invention's method  | 19            | 0.98       | 1.31                       | 187                     | -0.37              | 1.24       | 1.30                       | 273                     | -0.40                                                                                                      | -6.7      | -7.6        | -9.0  |
| Conventional method |               | 0.96       | 1.19                       | 176                     | -0.45              | 1.22       | 1.18                       | 263                     | -0.48                                                                                                      | -7.8      | -10.5       | -15.5 |
| Invention's method  | 20            | 0.95       | 1.27                       | 173                     | -0.38              | 1.20       | 1.26                       | 256                     | -0.41                                                                                                      | -6.9      | -7.9        | -9.3  |
| Conventional method |               | 0.93       | 1.15                       | 164                     | -0.46              | 1.18       | 1.14                       | 247                     | -0.49                                                                                                      | -8.1      | -10.8       | -16.0 |

On the basis of the results shown in Table 1 and Table 15 to 18, the magnetic properties of the bonded magnets and the hot-pressed magnets produced by using the rare earth magnet powders produced by the present invention's methods 16 to 20, in which a hydrogen-containing raw material mixed powder was produced by adding a hydride powder to a hydrogen-

<sup>60</sup> absorbing rare earth magnet raw material powder, and this hydrogen-containing raw material mixed powder was subjected to hydrogen absorption-decomposition, showed improvements in both coercivity and remanence when compared with the magnetic properties of bonded magnets and <sup>65</sup> hot-pressed magnets produced by using the rare earth magnet

49

powders produced by the conventional methods 16 to 20 in which a hydrogen-containing raw material mixed powder was obtained by adding a hydride powder to a rare earth magnet raw material hydride powder obtained by hydrogen absorption followed by hydrogen absorption-decomposition, and this hydrogen-containing raw material mixed powder was diffusion heat-treated. Moreover, the temperature coefficient of the coercivity and the thermal demagnetizing rate were both small, indicating that each of the magnets obtained by the present invention's methods also had an excellent thermal stability.

## Example 5

The present invention's methods 21 to 25 were carried out as follows. Blocks obtained from ingots f to j in Table 1 were subjected to hydrogen absorption under the conditions shown in Table 19. Then, these blocks subjected to the hydrogen absorption were milled to the average particle diameters shown in Table 19 so as to produce hydrogen-absorbing rare earth magnet alloy raw material powders. To these rare earth magnet alloy raw material powders subjected to hydrogen absorption, a Dy hydride powder, a Tb hydride powder, or a Dy—Tb binary alloy hydride powder, each of which has an average particle diameter of 5  $\mu\text{m}$  was added at the amount shown in Table 19, and then mixed therewith so as to produce hydrogen-containing raw material mixed powders. The respective hydrogen-containing raw material mixed powders were then subjected to, in order, hydrogen absorption-decomposition under the conditions shown in Table 19; if necessary, intermediate heat treatment under the conditions shown in Table 19; if necessary, heat treatment in depressurized hydrogen under the conditions shown in Table 20; hydrogen desorption under the conditions shown in Table 20; forcibly cooling to room temperature with Ar gas; and then pulverizing to 300  $\mu\text{m}$  or below, thereby producing rare earth magnet powders.

## Conventional Example 5

Conventional methods 21 to 25 were carried out as follows. Blocks obtained from ingots f to j in Table 1 were subjected to hydrogen absorption under the same conditions as in Example 5 and shown in Table 19 followed by hydrogen absorption-decomposition under the same conditions as in Example 5 and shown in Table 19, and then were subjected to, in order, if necessary, heat treatment in depressurized hydrogen under the conditions shown in Table 20; forcibly cooling to room temperature in Ar gas; and then milling treatment to the average particle diameter shown in Table 20 so as to produce rare earth magnet raw material hydride powders. To these rare earth magnet raw material hydride powders, a Dy hydride powder, a Tb hydride powder, or a Dy—Tb binary alloy hydride powder, each of which has an average particle diameter of 5  $\mu\text{m}$ , was added at the amount shown in Table 20 and then mixed therewith so as to produce hydrogen-containing raw material mixed powders. Each of these hydrogen-containing raw material mixed powders was subjected to

50

diffusion heat-treating including heating in a vacuum followed by holding under the conditions shown in Table 20; hydrogen desorption under the conditions shown in Table 16; forcibly cooling to room temperature with Ar gas; and then pulverizing to 300  $\mu\text{m}$  or below, thereby producing rare earth magnet powders.

10 Each of the rare earth magnet powders obtained by using the present invention's methods 21 to 25 and the conventional methods 21 to 25 was embedded in a phenolic resin and polished to a mirror surface, and the detected intensities of near-center and near-surface Dy and/or Tb, and the intensity ratio thereof were measured by analysis with the EPMA, thereby determining the values of the depth of the Dy—Tb rich layer from the surface and of the surface coverage by the Dy—Tb rich layer. Those results are given in Table 21.

15 In addition, to each of the rare earth magnet powders obtained in the present invention's methods 21 to 25 and the conventional methods 21 to 25, an epoxy resin was added at 3 wt % and then mixed therewith, and each of the mixtures was compression-molded in a magnetic field of 1.6 MA/m so as to produce a green compact. The green compact was hardened in an oven at 150° C. for 2 hours so as to produce a 20 bonded magnet having a density of 6.0 to 6.1 g/cm<sup>3</sup>. The magnetic properties of the obtained bonded magnet are 25 shown in Table 22. Also, the temperature coefficient of coercivity  $\alpha_{iHc}$  for each magnet was determined from the result of the magnetic properties measured at 150° C., and those values are 30 shown in Table 22.

Also, to each of the rare earth magnet powders obtained in the present invention's methods 21 to 25 and the conventional methods 21 to 25, an epoxy resin was added at 3 wt % and then 35 mixed therewith, and each of the mixtures was compression-molded while applying a magnetic field of 1.6 MA/m in a compacting direction so as to produce a green compact with a cylindrical shape having a diameter of 10 mm and a height of 7 mm. Subsequently, the obtained cylindrical green compact was hardened in an oven at 150° C. for 2 hours so as to 40 produce a cylindrical bonded magnet having a density of 6.0 to 6.1 g/cm<sup>3</sup>. To determine their magnetic properties, the obtained bonded magnet was magnetized in pulsed magnetic field of a 70 kOe, and then held for 1,000 hours in an oven maintained at 100° C., and the thermal demagnetizing rates after 3 hours, 100 hours, and 1,000 hours were measured. Those results are shown in Table 22, and the thermal 45 stability was evaluated.

50 In addition, the rare earth magnet powders obtained by using the present invention's method 21 to 25 and the conventional methods 21 to 25 were compression-molded in a magnetic field to produce anisotropic green compacts. These 55 anisotropic green compacts were set in a hot-pressing apparatus, and hot pressing was carried out under the following conditions: pressing in parallel to the magnetic aligned direction; an Ar gas atmosphere; a temperature of 750° C.; a pressure of 58.8 MPa; and holding time of 1 minute. The hot 60 pressing was following by quenching so as to produce hot-pressed magnets having a density of 7.5 to 7.7 g/cm<sup>3</sup>. The magnetic properties of the obtained hot-pressed magnets are 65 shown in Table 22. Also, the temperature coefficient of coercivity  $\alpha_{iHc}$  was determined from the result of the magnetic properties measured at 150° C., and those values are shown in Table 22.

TABLE 19

| Type                | Ingot in Table 1 | Hydrogen pressure (kPa) | Holding temp. (° C.) | Holding time (min) | Table 1 in Ar atmosphere (μm) | Average particle diameter of rare earth magnet raw material powder obtained by milling ingot in | Hydrogen-containing raw material mixed powder |            |                     | Hydrogen absorption-decomposition             |                      |                    | Intermediate heat treatment       |                      |                    |
|---------------------|------------------|-------------------------|----------------------|--------------------|-------------------------------|-------------------------------------------------------------------------------------------------|-----------------------------------------------|------------|---------------------|-----------------------------------------------|----------------------|--------------------|-----------------------------------|----------------------|--------------------|
|                     |                  |                         |                      |                    |                               |                                                                                                 | Dy hydride                                    | Tb hydride | Dy-Tb alloy hydride | Hydrogen pressure (kPa)                       | Holding temp. (° C.) | Holding time (min) | Ar pressure (kPa)                 | Holding temp. (° C.) | Holding time (min) |
|                     |                  |                         |                      |                    |                               |                                                                                                 | Hydrogen absorption                           |            |                     | Hydrogen-containing raw material mixed powder |                      |                    | Hydrogen absorption-decomposition |                      |                    |
| Invention's method  | 21               | f                       | 500                  | 150                | 20                            | 300                                                                                             | 0.1                                           | —          | —                   | 500                                           | 820                  | 120                | 500                               | 820                  | 5                  |
| Conventional method |                  |                         |                      |                    |                               | —                                                                                               | —                                             | —          | —                   | —                                             | —                    | —                  | —                                 | —                    | —                  |
| Invention's method  | 22               | g                       | 300                  | 180                | 40                            | 300                                                                                             | —                                             | 1.0        | —                   | 300                                           | 820                  | 240                | —                                 | —                    | —                  |
| Conventional method |                  |                         |                      |                    |                               | —                                                                                               | —                                             | —          | —                   | —                                             | —                    | —                  | —                                 | —                    | —                  |
| Invention's method  | 23               | h                       | 700                  | 200                | 60                            | 300                                                                                             | —                                             | —          | 2.0                 | 700                                           | 840                  | 180                | 700                               | 840                  | 10                 |
| Conventional method |                  |                         |                      |                    |                               | —                                                                                               | —                                             | —          | —                   | —                                             | —                    | —                  | —                                 | —                    | —                  |
| Invention's method  | 24               | i                       | 100                  | 250                | 90                            | 300                                                                                             | 3.0                                           | —          | —                   | 100                                           | 860                  | 60                 | —                                 | —                    | —                  |
| Conventional method |                  |                         |                      |                    |                               | —                                                                                               | —                                             | —          | —                   | —                                             | —                    | —                  | —                                 | —                    | —                  |
| Invention's method  | 25               | j                       | 900                  | 300                | 120                           | 300                                                                                             | —                                             | 5.0        | —                   | 900                                           | 880                  | 120                | 900                               | 880                  | 8                  |
| Conventional method |                  |                         |                      |                    |                               | —                                                                                               | —                                             | —          | —                   | —                                             | —                    | —                  | —                                 | —                    | —                  |

TABLE 20

| Type                | Remarks | Heat treatment in pressure-reduced hydrogen |                      |                    | Average particle diameter of rare earth magnet raw material hydride powder obtained by hydrogen absorption-decomposition, optionally heat treating in depressurized hydrogen, and then milling ingot in Table 1 (μm) | Hydrogen-containing raw material mixed powder |            |                     | Hydrogen absorption-decomposition, optionally heat treating in depressurized hydrogen, and then milling ingot in Table 1 (μm) | Hydrogen-containing raw material mixed powder                                    |   |   |  |  |
|---------------------|---------|---------------------------------------------|----------------------|--------------------|----------------------------------------------------------------------------------------------------------------------------------------------------------------------------------------------------------------------|-----------------------------------------------|------------|---------------------|-------------------------------------------------------------------------------------------------------------------------------|----------------------------------------------------------------------------------|---|---|--|--|
|                     |         | Hydrogen Pressure (kPa)                     | Holding temp. (° C.) | Holding time (min) |                                                                                                                                                                                                                      | Dy hydride                                    | Tb hydride | Dy-Tb alloy hydride |                                                                                                                               | Amount of hydride added to rare earth magnet raw material hydride powder (mol %) |   |   |  |  |
|                     |         |                                             |                      |                    |                                                                                                                                                                                                                      | Heat treatment in pressure-reduced hydrogen   |            |                     |                                                                                                                               |                                                                                  |   |   |  |  |
| Invention's method  | 21      | Cont'd from Table 19                        | 2.6                  | 820                | 120                                                                                                                                                                                                                  | —                                             | —          | —                   | —                                                                                                                             | —                                                                                | — | — |  |  |
| Conventional method |         |                                             |                      |                    |                                                                                                                                                                                                                      | 300                                           | 0.1        | —                   | —                                                                                                                             | —                                                                                | — | — |  |  |
| Invention's method  | 22      |                                             | 3.9                  | 820                | 120                                                                                                                                                                                                                  | —                                             | —          | —                   | —                                                                                                                             | —                                                                                | — | — |  |  |
| Conventional method |         |                                             |                      |                    |                                                                                                                                                                                                                      | 300                                           | —          | 1                   | —                                                                                                                             | —                                                                                | — | — |  |  |
| Invention's method  | 23      |                                             | —                    |                    |                                                                                                                                                                                                                      | —                                             | —          | —                   | —                                                                                                                             | —                                                                                | — | — |  |  |
| Conventional method |         |                                             | 3.9                  | 840                | 120                                                                                                                                                                                                                  | 300                                           | —          | —                   | 2                                                                                                                             | —                                                                                | — | — |  |  |
| Invention's method  | 24      |                                             | —                    |                    |                                                                                                                                                                                                                      | —                                             | —          | —                   | —                                                                                                                             | —                                                                                | — | — |  |  |
| Conventional method |         |                                             | 3.9                  | 860                | 120                                                                                                                                                                                                                  | 300                                           | 3          | —                   | —                                                                                                                             | —                                                                                | — | — |  |  |
| Invention's method  | 25      |                                             | 8                    | 880                | 240                                                                                                                                                                                                                  | —                                             | —          | —                   | —                                                                                                                             | —                                                                                | — | — |  |  |
| Conventional method |         |                                             |                      |                    |                                                                                                                                                                                                                      | 300                                           | —          | 5                   | —                                                                                                                             | —                                                                                | — | — |  |  |

TABLE 20-continued

| Type                   | Remarks | Diffusion heat-treatment |                            |                          | Hydrogen desorption           |                            |                          |
|------------------------|---------|--------------------------|----------------------------|--------------------------|-------------------------------|----------------------------|--------------------------|
|                        |         | Pressure<br>(kPa)        | Holding<br>temp.<br>(° C.) | Holding<br>time<br>(min) | Ultimate<br>Pressure<br>(kPa) | Holding<br>temp.<br>(° C.) | Holding<br>time<br>(min) |
|                        |         |                          |                            |                          |                               |                            |                          |
| Invention's<br>method  | 21      |                          | —                          |                          | 0.066                         | 820                        | 12                       |
| Conventional<br>method |         | $1 \times 10^{-4}$       | 820                        | 30                       | $1 \times 10^{-4}$            |                            | 30                       |
| Invention's<br>method  | 22      |                          | —                          |                          | 0.026                         | 820                        | 16                       |
| Conventional<br>method |         | $1 \times 10^{-4}$       | 820                        | 30                       | $1 \times 10^{-4}$            |                            | 30                       |
| Invention's<br>method  | 23      |                          | —                          |                          | 0.013                         | 840                        | 9                        |
| Conventional<br>method |         | $1 \times 10^{-4}$       | 840                        | 30                       | $1 \times 10^{-4}$            |                            | 30                       |
| Invention's<br>method  | 24      |                          | —                          |                          | 0.013                         | 860                        | 7                        |
| Conventional<br>method |         | $1 \times 10^{-4}$       | 860                        | 30                       | $1 \times 10^{-4}$            |                            | 30                       |
| Invention's<br>method  | 25      |                          | —                          |                          | 0.013                         | 880                        | 10                       |
| Conventional<br>method |         | $1 \times 10^{-4}$       | 880                        | 30                       | $1 \times 10^{-4}$            |                            | 30                       |

TABLE 21

| Type                   | Remarks | Rare earth magnet powder                  |                                          |                    |                                         |                 |     |
|------------------------|---------|-------------------------------------------|------------------------------------------|--------------------|-----------------------------------------|-----------------|-----|
|                        |         | EPMA detected intensity                   |                                          |                    | Thickness                               |                 |     |
|                        |         | Peak<br>value<br>near surface<br>(counts) | Peak<br>value<br>near center<br>(counts) | Intensity<br>ratio | of<br>Dy—Tb<br>rich layer<br>( $\mu$ m) | Coverage<br>(%) |     |
| Invention's<br>method  | 21      | Continued<br>from<br>Table 20             | 1880                                     | 1446               | 1.24                                    | 0.2             | 75  |
| Conventional<br>method |         |                                           | 1447                                     | 1492               | 0.97                                    | —               | 0   |
| Invention's<br>method  | 22      |                                           | 3377                                     | 1777               | 1.90                                    | 7.0             | 90  |
| Conventional<br>method |         |                                           | 2367                                     | 2233               | 1.06                                    | —               | 0   |
| Invention's<br>method  | 23      |                                           | 2771                                     | 947                | 2.94                                    | 10.9            | 100 |
| Conventional<br>method |         |                                           | 2076                                     | 1854               | 1.12                                    | —               | 0   |
| Invention's<br>method  | 24      |                                           | 4492                                     | 1140               | 3.94                                    | 21.9            | 100 |
| Conventional<br>method |         |                                           | 2274                                     | 1960               | 1.16                                    | —               | 0   |
| Invention's<br>method  | 25      |                                           | 17790                                    | 3646               | 4.88                                    | 27.1            | 100 |
| Conventional<br>method |         |                                           | 7286                                     | 5923               | 1.23                                    | 1.0             | 20  |

TABLE 22

| Type                | Bonded magnet |            |                            |                         | Hot-pressed magnet |            |                            |                         | Thermal demagnetizing rate for bonded magnet after being held for time indicated below in 100° C. oven (%) |           |             |       |
|---------------------|---------------|------------|----------------------------|-------------------------|--------------------|------------|----------------------------|-------------------------|------------------------------------------------------------------------------------------------------------|-----------|-------------|-------|
|                     | Br (T)        | iHc (MA/m) | BHmax (KJ/m <sup>3</sup> ) | $\alpha_{iHc}$ (%/° C.) | Br (T)             | iHc (MA/m) | BHmax (KJ/m <sup>3</sup> ) | $\alpha_{iHc}$ (%/° C.) | 3 hours                                                                                                    | 100 hours | 1,000 hours |       |
| Invention's method  | 21            | 0.93       | 1.74                       | 159                     | -0.40              | 1.18       | 1.73                       | 247                     | -0.43                                                                                                      | -5.0      | -5.7        | -6.8  |
| Conventional method |               | 0.91       | 1.73                       | 149                     | -0.41              | 1.15       | 1.71                       | 236                     | -0.44                                                                                                      | -5.4      | -7.2        | -10.7 |
| Invention's method  | 22            | 0.95       | 1.78                       | 167                     | -0.38              | 1.20       | 1.76                       | 256                     | -0.41                                                                                                      | -4.9      | -5.6        | -6.7  |
| Conventional method |               | 0.93       | 1.66                       | 158                     | -0.43              | 1.18       | 1.65                       | 247                     | -0.46                                                                                                      | -5.6      | -7.5        | -11.1 |
| Invention's method  | 23            | 0.95       | 1.47                       | 173                     | -0.36              | 1.21       | 1.46                       | 260                     | -0.39                                                                                                      | -6.0      | -6.8        | -8.1  |
| Conventional method |               | 0.94       | 1.25                       | 165                     | -0.42              | 1.19       | 1.24                       | 252                     | -0.45                                                                                                      | -7.5      | -10.0       | -14.8 |
| Invention's method  | 24            | 0.94       | 1.51                       | 166                     | -0.35              | 1.19       | 1.50                       | 253                     | -0.37                                                                                                      | -5.8      | -6.6        | -7.8  |
| Conventional method |               | 0.93       | 1.39                       | 160                     | -0.41              | 1.18       | 1.38                       | 247                     | -0.44                                                                                                      | -6.7      | -9.0        | -13.3 |
| Invention's method  | 25            | 0.96       | 2.51                       | 166                     | -0.34              | 1.22       | 2.49                       | 266                     | -0.36                                                                                                      | -3.5      | -4.0        | -4.7  |
| Conventional method |               | 0.96       | 2.04                       | 164                     | -0.40              | 1.22       | 2.02                       | 263                     | -0.43                                                                                                      | -4.6      | -6.1        | -9.1  |

On the basis of the results shown in Table 1 and Table 19 to 22, the magnetic properties of the bonded magnets and the hot-pressed magnets produced by using the rare earth magnet powders produced by the present invention's methods 21 to 25, in which a hydrogen-containing raw material mixed powder was produced by adding a hydride powder to a hydrogen-absorbing rare earth magnet raw material powder, and this hydrogen-containing raw material mixed powder was subjected to hydrogen absorption-decomposition, showed improvements in both coercivity and remanence when compared with the magnetic properties of bonded magnets and hot-pressed magnets produced by using the rare earth magnet powders produced by the conventional methods 21 to 25 in which a hydrogen-containing raw material mixed powder was obtained by adding a hydride powder to a rare earth magnet raw material hydride powder obtained by hydrogen absorption followed by hydrogen absorption-decomposition, and this hydrogen-containing raw material mixed powder was diffusion heat-treated. Moreover, the temperature coefficient of the coercivity and the thermal demagnetizing rate were both small, indicating that each of the magnets obtained by the present invention's methods also had an excellent thermal stability.

#### Example 6

The present invention's methods 26 to 30 were carried out as follows. Blocks obtained from ingots k to o in Table 1 was subjected to hydrogen absorption under the conditions shown in Table 23. Then, these blocks subjected to the hydrogen absorption were milled to the average particle diameters shown in Table 23 so as to produce hydrogen-absorbing rare earth magnet alloy raw material powders. To these rare earth magnet alloy raw material powders subjected to hydrogen absorption, a Dy hydride powder, a Tb hydride powder, or a Dy—Tb binary alloy hydride powder, each of which has an average particle diameter of 5  $\mu\text{m}$  was added at the amount

30 shown in Table 19, and then mixed therewith so as to produce hydrogen-containing raw material mixed powders. The respective hydrogen-containing raw material mixed powders were then subjected to, in order, hydrogen absorption-decomposition under the conditions shown in Table 23; if necessary, intermediate heat treatment under the conditions shown in Table 23; if necessary, heat treatment in depressurized hydrogen under the conditions shown in Table 23; hydrogen desorption under the conditions shown in Table 24; forcibly cooling to room temperature with Ar gas; and then pulverizing to 300  $\mu\text{m}$  or below, thereby producing rare earth magnet powders.

#### Conventional Example 6

45 Conventional methods 26 to 30 were carried out as follows. Blocks obtained from ingots k to o in Table 1 were subjected to hydrogen absorption under the same conditions as in Example 6 and shown in Table 23 followed by hydrogen absorption-decomposition under the same conditions as in Example 6 and shown in Table 23 without milling the blocks nor adding a hydride powder so as not to produce a hydrogen-containing raw material mixed powder, and then were subjected to, in order, if necessary, heat treatment in depressurized 50 hydrogen under the conditions shown in Table 23; forcibly cooling to room temperature in Ar gas; and then milling treatment to the average particle diameter shown in Table 24 so as to produce rare earth magnet raw material hydride powders. To these rare earth magnet raw material hydride powders, a Dy hydride powder, a Tb hydride powder, or a Dy—Tb binary alloy hydride powder, each of which has an average particle diameter of 5  $\mu\text{m}$ , was added at the amount shown in Table 24 and then mixed therewith so as to produce 55 hydrogen-containing raw material mixed powders. Each of these hydrogen-containing raw material mixed powders was subjected to diffusion heat-treating including heating in a vacuum followed by holding under the conditions shown in 60

65

Table 24; hydrogen desorption under the conditions shown in Table 24; forcibly cooling to room temperature with Ar gas; and then pulverizing to 300  $\mu\text{m}$  or below, thereby producing rare earth magnet powders.

Each of the rare earth magnet powders obtained by using the present invention's methods 26 to 30 and the conventional methods 26 to 30 was embedded in a phenolic resin and polished to a mirror surface, and the detected intensities of near-center and near-surface Dy and/or Tb, and the intensity ratio thereof were measured by analysis with the EPMA, thereby determining the values of the depth of the Dy—Tb rich layer from the surface and of the surface coverage by the Dy—Tb rich layer. Those results are given in Table 25.

To each of the rare earth magnet powders obtained in the present invention's methods 26 to 30 and the conventional methods 26 to 30, an epoxy resin was added at 3 wt % and then mixed therewith, and each of the mixtures was compression-molded in a magnetic field of 1.6 MA/m so as to produce a green compact. The green compact was hardened in an oven at 150° C. for 2 hours so as to produce a bonded magnet having a density of 6.0 to 6.1 g/cm<sup>3</sup>. The magnetic properties of the obtained bonded magnet are shown in Table 26. Also, the temperature coefficient of coercivity  $\alpha_{iHc}$  for each magnet was determined from the result of the magnetic properties measured at 150° C., and those values are shown in Table 26.

Also, to each of the rare earth magnet powders obtained in the present invention's methods 26 to 30 and the conventional methods 26 to 30, an epoxy resin was added at 3 wt % and then mixed therewith, and each of the mixtures was compression-

molded while applying a magnetic field of 1.6 MA/m in a compacting direction so as to produce a green compact with a cylindrical shape having a diameter of 10 mm and a height of 7 mm. Subsequently, the obtained cylindrical green compact was hardened in an oven at 150° C. for 2 hours so as to produce a cylindrical bonded magnet having a density of 6.0 to 6.1 g/cm<sup>3</sup>. To determine their magnetic properties, the obtained bonded magnet was magnetized in pulsed magnetic field of a 70 kOe, and then held for 1,000 hours in an oven maintained at 100° C., and the thermal demagnetizing rates after 3 hours, 100 hours, and 1,000 hours were measured. Those results are shown in Table 26, and the thermal stability was evaluated.

In addition, the rare earth magnet powders obtained by using the present invention's method 26 to 30 and the conventional methods 26 to 30 were compression-molded in a magnetic field to produce anisotropic green compacts. These anisotropic green compacts were set in a hot-pressing apparatus, and hot pressing was carried out under the following conditions: pressing in parallel to the magnetic aligned direction; an Ar gas atmosphere; a temperature of 750° C.; a pressure of 58.8 MPa; and holding time of 1 minute. The hot pressing was followed by quenching so as to produce hot-pressed magnets having a density of 7.5 to 7.7 g/cm<sup>3</sup>. The magnetic properties of the obtained hot-pressed magnets are shown in Table 26. Also, the temperature coefficient of coercivity  $\alpha_{iHc}$  was determined from the result of the magnetic properties measured at 150° C., and those values are shown in Table 26.

TABLE 23

| Type                   | Ingot                                   |   | Table 1 in<br>Ar atmosphere ( $\mu\text{m}$ ) | Dy hydride | Tb hydride | Dy—Tb alloy | Hydrogen                                    | Intermediate heat treatment                                                                       |     |   | Heat treatment in<br>depressurized hydrogen |     |     |  |  |  |  |  |
|------------------------|-----------------------------------------|---|-----------------------------------------------|------------|------------|-------------|---------------------------------------------|---------------------------------------------------------------------------------------------------|-----|---|---------------------------------------------|-----|-----|--|--|--|--|--|
|                        | in<br>Table 1<br>Hydrogen<br>absorption |   |                                               |            |            |             |                                             | Mixed powder<br>Amount of hydride<br>added to rare earth<br>magnet raw material<br>powder (mol %) |     |   | Ar pressure<br>(kPa)                        |     |     |  |  |  |  |  |
|                        |                                         |   |                                               |            |            |             |                                             |                                                                                                   |     |   |                                             |     |     |  |  |  |  |  |
| Invention's<br>method  | 26                                      | k | Hydrogen<br>partial<br>pressure:<br>200 kPa   | 10         | 0.5        | —           | Hydrogen<br>partial<br>pressure:<br>200 kPa | 200                                                                                               | 820 | 5 | 3.9                                         | 820 | 120 |  |  |  |  |  |
| Conventional<br>method | 27                                      | 1 | Holding<br>temp.:<br>150° C.                  | 50         | —          | —           | Holding<br>temp.:<br>820° C.                | —                                                                                                 | —   | — | 3.9                                         | 820 | 120 |  |  |  |  |  |
| Invention's<br>method  | 28                                      | m | Holding<br>time:<br>20 min                    | 100        | 1.0        | 1.0         | Hydrogen<br>partial<br>pressure:<br>200 kPa | 200                                                                                               | 820 | 5 | —                                           | —   | —   |  |  |  |  |  |
| Conventional<br>method |                                         |   |                                               | —          | —          | —           | Holding<br>time:<br>120 min                 | —                                                                                                 | —   | — | 3.9                                         | 820 | 120 |  |  |  |  |  |
| Invention's<br>method  | 29                                      | n |                                               | 200        | —          | 2.0         | 2.0                                         | —                                                                                                 | —   | — | —                                           | —   | —   |  |  |  |  |  |
| Conventional<br>method |                                         |   |                                               | —          | —          | —           |                                             |                                                                                                   |     |   | 3.9                                         | 820 | 120 |  |  |  |  |  |
| Invention's<br>method  | 30                                      | o |                                               | 500        | 2.0        | —           | —                                           | 200                                                                                               | 820 | 5 | 3.9                                         | 820 | 120 |  |  |  |  |  |
| Conventional<br>method |                                         |   |                                               | —          | —          | —           |                                             | —                                                                                                 | —   | — |                                             |     |     |  |  |  |  |  |

TABLE 24

| Type                | Remarks                    | Average particle diameter of rare earth magnet raw material hydride powder obtained by heat-treating ingot in Table 1 in depressurized | Hydrogen-containing raw material |            |            | Diffusion heat-treatment |                      |                      | Hydrogen desorption |                         |                      |                    |
|---------------------|----------------------------|----------------------------------------------------------------------------------------------------------------------------------------|----------------------------------|------------|------------|--------------------------|----------------------|----------------------|---------------------|-------------------------|----------------------|--------------------|
|                     |                            |                                                                                                                                        | hydrogen, then milling (μm)      | Dy hydride | Tb hydride | Dy—Tb alloy hydride      | Pressure (kPa)       | Holding temp. (° C.) | Holding time (min)  | Ultimate pressure (kPa) | Holding temp. (° C.) | Holding time (min) |
| Invention's method  | 26 Continued from Table 23 | —                                                                                                                                      | —                                | —          | —          | —                        | —                    | —                    | —                   | 0.013                   | 820                  | 8                  |
| Conventional method |                            | 10                                                                                                                                     | 0.5                              | —          | —          | —                        | 1 × 10 <sup>-4</sup> | 820                  | 30                  | 1 × 10 <sup>-4</sup>    |                      | 30                 |
| Invention's method  | 27                         | —                                                                                                                                      | —                                | —          | —          | —                        | —                    | —                    | —                   | 0.013                   |                      | 13                 |
| Conventional method |                            | 50                                                                                                                                     | —                                | —          | —          | 1.5                      | 1 × 10 <sup>-4</sup> | 820                  | 30                  | 1 × 10 <sup>-4</sup>    |                      | 30                 |
| Invention's method  | 28                         | —                                                                                                                                      | —                                | —          | —          | —                        | —                    | —                    | —                   | 0.013                   |                      | 7                  |
| Conventional method |                            | 100                                                                                                                                    | 1                                | 1          | —          | —                        | 1 × 10 <sup>-4</sup> | 820                  | 30                  | 1 × 10 <sup>-4</sup>    |                      | 30                 |
| Invention's method  | 29                         | —                                                                                                                                      | —                                | —          | —          | —                        | —                    | —                    | —                   | 0.013                   |                      | 9                  |
| Conventional method |                            | 200                                                                                                                                    | —                                | 2          | 2          | —                        | 1 × 10 <sup>-4</sup> | 820                  | 30                  | 1 × 10 <sup>-4</sup>    |                      | 30                 |
| Invention's method  | 30                         | —                                                                                                                                      | —                                | —          | —          | —                        | —                    | —                    | —                   | 0.013                   |                      | 12                 |
| Conventional method |                            | 500                                                                                                                                    | 2                                | —          | —          | —                        | 1 × 10 <sup>-4</sup> | 820                  | 30                  | 1 × 10 <sup>-4</sup>    |                      | 30                 |

TABLE 25

| Type                | Remarks                    | Rare earth magnet powder         |                                 |                 |                          |              |  |
|---------------------|----------------------------|----------------------------------|---------------------------------|-----------------|--------------------------|--------------|--|
|                     |                            | EPMA detected intensity          |                                 |                 | Thickness                |              |  |
|                     |                            | Peak value near surface (counts) | Peak value near center (counts) | Intensity ratio | of Dy—Tb rich layer (μm) | Coverage (%) |  |
| Invention's method  | 26 Continued from Table 24 | 2363                             | 1524                            | 1.55            | 4.9                      | 90           |  |
| Conventional method |                            | 1760                             | 1752                            | 1.00            | —                        | 0            |  |
| Invention's method  | 27                         | 2974                             | 1383                            | 2.15            | 8.0                      | 100          |  |
| Conventional method |                            | 2253                             | 2067                            | 1.09            | —                        | 0            |  |
| Invention's method  | 28                         | 2654                             | 1270                            | 2.09            | 11.6                     | 100          |  |
| Conventional method |                            | 2017                             | 1817                            | 1.11            | —                        | 0            |  |
| Invention's method  | 29                         | 8711                             | 2257                            | 3.86            | 21.4                     | 100          |  |
| Conventional method |                            | 4054                             | 3350                            | 1.21            | 0.5                      | 10           |  |
| Invention's method  | 30                         | 2939                             | 893                             | 3.29            | 12.2                     | 100          |  |
| Conventional method |                            | 1627                             | 1440                            | 1.13            | —                        | 0            |  |

TABLE 26

| Type                | Bonded magnet |            |                            |                         | Hot-pressed magnet |            |                            |                         | Thermal demagnetizing rate for bonded magnet after being held for time indicated below in 100° C. oven (%) |           |             |       |
|---------------------|---------------|------------|----------------------------|-------------------------|--------------------|------------|----------------------------|-------------------------|------------------------------------------------------------------------------------------------------------|-----------|-------------|-------|
|                     | Br (T)        | iHc (MA/m) | BHmax (KJ/m <sup>3</sup> ) | $\alpha_{iHc}$ (%/° C.) | Br (T)             | iHc (MA/m) | BHmax (KJ/m <sup>3</sup> ) | $\alpha_{iHc}$ (%/° C.) | 3 hours                                                                                                    | 100 hours | 1,000 hours |       |
| Invention's method  | 26            | 0.95       | 1.69                       | 161                     | -0.39              | 1.20       | 1.68                       | 257                     | -0.42                                                                                                      | -5.2      | -5.9        | -7.0  |
| Conventional method |               | 0.93       | 1.61                       | 152                     | -0.42              | 1.18       | 1.59                       | 247                     | -0.45                                                                                                      | -5.8      | -7.8        | -11.5 |
| Invention's method  | 27            | 0.94       | 1.72                       | 159                     | -0.37              | 1.18       | 1.70                       | 250                     | -0.40                                                                                                      | -5.1      | -5.8        | -6.9  |
| Conventional method |               | 0.92       | 1.58                       | 150                     | -0.43              | 1.17       | 1.56                       | 242                     | -0.46                                                                                                      | -5.9      | -7.9        | -11.7 |
| Invention's method  | 28            | 0.96       | 1.46                       | 172                     | -0.36              | 1.22       | 1.44                       | 265                     | -0.39                                                                                                      | -6.0      | -6.9        | -8.1  |
| Conventional method |               | 0.95       | 1.31                       | 165                     | -0.44              | 1.20       | 1.30                       | 258                     | -0.47                                                                                                      | -7.1      | -9.5        | -14.1 |
| Invention's method  | 29            | 0.95       | 2.11                       | 166                     | -0.36              | 1.20       | 2.09                       | 257                     | -0.39                                                                                                      | -4.1      | -4.7        | -5.6  |
| Conventional method |               | 0.94       | 1.79                       | 161                     | -0.43              | 1.19       | 1.77                       | 252                     | -0.46                                                                                                      | -5.3      | -7.0        | -10.3 |
| Invention's method  | 30            | 0.97       | 1.42                       | 180                     | -0.36              | 1.23       | 1.41                       | 271                     | -0.39                                                                                                      | -6.2      | -7.0        | -8.3  |
| Conventional method |               | 0.96       | 1.23                       | 172                     | -0.45              | 1.22       | 1.22                       | 263                     | -0.48                                                                                                      | -7.6      | -10.1       | -15.0 |

On the basis of the results shown in Table 1 and Table 23 to 26, the magnetic properties of the bonded magnets and the hot-pressed magnets produced by using the rare earth magnet powders produced by the present invention's methods 26 to 30, in which a hydrogen-containing raw material mixed powder was produced by adding a hydride powder to a hydrogen-absorbing rare earth magnet raw material powder, and this hydrogen-containing raw material mixed powder was subjected to hydrogen absorption-decomposition, showed improvements in both coercivity and remanence when compared with the magnetic properties of bonded magnets and hot-pressed magnets produced by using the rare earth magnet powders produced by the conventional methods 26 to 30 in which a hydrogen-containing raw material mixed powder was obtained by adding a hydride powder to a rare earth magnet raw material hydride powder obtained by hydrogen absorption followed by hydrogen absorption-decomposition, and this hydrogen-containing raw material mixed powder was diffusion heat-treated. Moreover, the temperature coefficient of the coercivity and the thermal demagnetizing rate were both small, indicating that each of the magnets obtained by the present invention's methods also had an excellent thermal stability.

#### INDUSTRIAL APPLICABILITY

The rare earth magnet powders obtained by the methods of producing a rare earth magnet powder of the present invention are excellent in magnetic anisotropy and thermal stability, and thus exhibit outstanding effects in industrial use.

The invention claimed is:

1. A rare earth magnet powder comprising:  
a chemical composition comprising R: 5 to 20 atom % (wherein R represents one, or two or more rare earth elements being inclusive of Y but exclusive of Dy and Tb), one or both of Dy and Tb: 0.01 to 10 atom %, B: 3 to 20 atom %, and M: 0.001 to 5 atom % (wherein M represents one, or two or more from among Ga, Zr, Nb, Mo, Hf, Ta, W, Ni, Al, Ti, V, Cu, Cr, Ge, C, and Si), with the balance comprising Fe and inevitable impurities, an average particle diameter being 10 to 1,000  $\mu\text{m}$ , wherein 60  
70% or more of the entire surface of the rare earth magnet powder is covered with a Dy—Tb rich layer being rich in content of the one or both of Dy and Tb and having a thickness of 0.05 to 50  $\mu\text{m}$ , and  
a concentration of the one or both of Dy and Tb in the Dy—Tb rich layer is such that the maximum detected intensity of the one or both of Dy and Tb, as measured by wavelength dispersive X-ray spectroscopy, is 1.2 to 5 times the average detected intensity in the central portion being present in the range of  $\frac{1}{3}$  of the particle diameter of a particle of the rare earth magnet powder.

3 to 20 atom %, with the balance comprising Fe and inevitable impurities, an average particle diameter being 10 to 1,000  $\mu\text{m}$ , wherein

35  
70% or more of the entire surface of the rare earth magnet powder is covered with a Dy—Tb rich layer being rich in content of the one or both of Dy and Tb and having a thickness of 0.05 to 50  $\mu\text{m}$ , and  
a concentration of the one or both of Dy and Tb in the Dy—Tb rich layer is such that the maximum detected intensity of the one or both of Dy and Tb, as measured by wavelength dispersive X-ray spectroscopy, is 1.2 to 5 times the average detected intensity in the central portion being present in the range of  $\frac{1}{3}$  of the particle diameter of a particle of the rare earth magnet powder.

40  
2. A rare earth magnet powder comprising:  
a chemical composition comprising R: 5 to 20 atm % (wherein R represents one, or two or more rare earth elements being inclusive of Y but exclusive of Dy and Tb), one or both of Dy and Tb: 0.01 to 10 atm %, B: 3 to 20 atm %, and M: 0.001 to 5 atm % (wherein M represents one, or two or more from among Ga, Zr, Nb, Mo, Hf, Ta, W, Ni, Al, Ti, V, Cu, Cr, Ge, C, and Si), with the balance comprising Fe and inevitable impurities, an average particle diameter being 10 to 1,000  $\mu\text{m}$ , wherein  
70% or more of the entire surface of the rare earth magnet powder is covered with a Dy—Tb rich layer being rich in content of the one or both of Dy and Tb and having a thickness of 0.05 to 50  $\mu\text{m}$ , and  
a concentration of the one or both of Dy and Tb in the Dy—Tb rich layer is such that the maximum detected intensity of the one or both of Dy and Tb, as measured by wavelength dispersive X-ray spectroscopy, is 1.2 to 5 times the average detected intensity in the central portion being present in the range of  $\frac{1}{3}$  of the particle diameter of a particle of the rare earth magnet powder.

45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
67

## 63

3. A rare earth magnet powder comprising:  
a chemical composition comprising R: 5 to 20 atm % (wherein R represents one, or two or more rare earth elements being inclusive of Y but exclusive of Dy and Tb), Co: 0.1 to 50 atm %, one or both of Dy and Tb: 0.01 to 10 atm %, and B: 3 to 20 atm %, with the balance comprising Fe and inevitable impurities, an average particle diameter being 10 to 1,000  $\mu\text{m}$ , wherein

70% or more of the entire surface of the rare earth magnet powder is covered with a Dy—Tb rich layer being rich in content of the one or both of Dy and Tb and having a thickness of 0.05 to 50  $\mu\text{m}$ , and

a concentration of the one or both of Dy and Tb in the Dy—Tb rich layer is such that the maximum detected intensity of the one or both of Dy and Tb, as measured by wavelength dispersive X-ray spectroscopy, is 1.2 to 5 times the average detected intensity in the central portion being present in the range of  $\frac{1}{3}$  of the particle diameter of a particle of the rare earth magnet powder.

4. A rare earth magnet powder comprising:

a chemical composition comprising R: 5 to 20 atm % (wherein M represents one, or two or more from among Ga, Zr, Nb, Mo, Hf, Ta, W, Ni, Al, Ti, V, Cu, Cr, Ge, C, and Si), one or both of Dy and Tb: 0.01 to 10 atm %, Co: 0.1 to 50 atm %, B: 3 to 20 atm %, and M: 0.001 to 5 atm % (wherein M represents one, or two or more from among Ga, Zr, Nb, Mo, Hf, Ta, W, Ni, Al, Ti, V, Cu, Cr, Ge, C, and Si), with the balance comprising Fe and inevitable impurities, an average particle diameter being 10 to 1,000  $\mu\text{m}$ , wherein

70% or more of the entire surface of the rare earth magnet powder is covered with a Dy—Tb rich layer being rich in

## 64

content of the one or both of Dy and Tb and having a thickness of 0.05 to 50  $\mu\text{m}$ , and  
a concentration of the one or both of Dy and Tb in the Dy—Tb rich layer is such that the maximum detected intensity of the one or both of Dy and Tb, as measured by wavelength dispersive X-ray spectroscopy, is 1.2 to 5 times the average detected intensity in the central portion being present in the range of  $\frac{1}{3}$  of the particle diameter of a particle of the rare earth magnet powder.

5. A rare earth magnet powder which is excellent in magnetic anisotropy and thermal stability according to any one of claims 1 to 4, further comprising:

a recrystallization texture in which recrystallized grains, whose main phase is a  $\text{R}_2\text{Fe}_{14}\text{B}$  intermetallic compound phase that is substantially a tetragonal structure, are adjacent to each other, wherein

the recrystallization texture comprises a basic texture of a magnetically anisotropic HDDR magnet powder in which the recrystallized grains, whose ratio (b/a) of a longest particle diameter (b) to a shortest particle diameter (a) is less than 2, exists at 50 vol % or more of all the recrystallized grains and an average recrystallized grain diameter of the recrystallized grains is 0.05 to 5  $\mu\text{m}$ .

6. A rare earth magnet produced by binding a rare earth magnet powder which is excellent in magnetic anisotropy and thermal stability according to any one of claims 1 to 4 with an organic binder or a metal binder.

7. A rare earth magnet produced by processing a rare earth magnet powder which is excellent in magnetic anisotropy and thermal stability according to any one of claims 1 to 4 with hot pressing or hot isostatic pressing.

\* \* \* \* \*